



US011739409B2

(12) **United States Patent**  
**Stowell et al.**

(10) **Patent No.:** US 11,739,409 B2  
(b4) **Date of Patent:** Aug. 29, 2023

(54) **APPARATUSES AND METHODS FOR PRODUCING COVETIC MATERIALS USING MICROWAVE REACTORS**

(71) Applicant: **LytEn, Inc.**, San Jose, CA (US)

(72) Inventors: **Michael W. Stowell**, Sunnyvale, CA (US); **Bruce Lanning**, Littleton, CO (US); **Peter Todd Williams**, San Carlos, CA (US); **Daniel Cook**, Woodside, CA (US)

(73) Assignee: **LytEn, Inc.**, San Jose, CA (US)

(\*) Notice: Subject to any disclaimer, the term of this patent is extended or adjusted under 35 U.S.C. 154(b) by 210 days.

(21) Appl. No.: 17/241,852

(22) Filed: **Apr. 27, 2021**

(65) **Prior Publication Data**

US 2021/0310110 A1 Oct. 7, 2021

**Related U.S. Application Data**

(60) Division of application No. 16/752,693, filed on Jan. 27, 2020, now abandoned, which is a (Continued)

(51) **Int. Cl.**  
**C23C 4/134** (2016.01)  
**H05H 1/30** (2006.01)  
(Continued)

(52) **U.S. Cl.**  
CPC ..... **C23C 4/067** (2016.01); **H05H 1/30** (2013.01); **H05H 1/461** (2021.05); **B22F 1/16** (2022.01);  
(Continued)

(58) **Field of Classification Search**

None  
See application file for complete search history.

(56) **References Cited**

U.S. PATENT DOCUMENTS

4,919,853 A \* 4/1990 Alvarez ..... B05B 7/0416  
261/DIG. 78  
4,991,541 A \* 2/1991 Sugata ..... C23C 16/54  
118/716

(Continued)

FOREIGN PATENT DOCUMENTS

WO 2012/158532 A1 11/2012  
WO 2017/177198 A1 10/2017

(Continued)

OTHER PUBLICATIONS

Extended European Search Report (EESR) issued in Appl. No. EP20790948.2 dated Oct. 5, 2022; 6 pages.

(Continued)

*Primary Examiner* — Binu Thomas

(74) *Attorney, Agent, or Firm* — Paradice & Li LLP

(57) **ABSTRACT**

Apparatuses and methods for producing covetic materials by exciting a hydrocarbon gas with pulse microwaves to form hydrocarbon radicals in a hot first region of a microwave reactor. Graphene nanoplatelets are formed by the nucleation, growth and assembly of the hydrocarbon radicals, and contact a metal melt introduced downstream of the hot region to produce a mixture of molten metal and graphene nanoplatelets which assemble in-flight to form covetic materials. Graphene planes are infused in the metal matrix to achieve carbon loadings of at least 60%.

**12 Claims, 49 Drawing Sheets**



**Related U.S. Application Data**

continuation-in-part of application No. 16/460,177, filed on Jul. 2, 2019, now abandoned.

2019/0283379 A1 9/2019 Lin et al.  
 2019/0381563 A1 12/2019 Balachandran et al.  
 2020/0223698 A1\* 7/2020 Kroeger ..... H05H 1/30

**FOREIGN PATENT DOCUMENTS**

WO 2017/180641 A2 10/2017  
 WO 2018/104689 A1 6/2018  
 WO 2018/126191 A1 7/2018  
 WO 2019/095039 A1 5/2019

**OTHER PUBLICATIONS**

- (60) Provisional application No. 62/903,649, filed on Sep. 20, 2019, provisional application No. 62/868,493, filed on Jun. 28, 2019, provisional application No. 62/839,995, filed on Apr. 29, 2019, provisional application No. 62/797,306, filed on Jan. 27, 2019, provisional application No. 62/720,677, filed on Aug. 21, 2018, provisional application No. 62/714,030, filed on Aug. 2, 2018.

**(51) Int. Cl.**

**H05H 1/46** (2006.01)  
**C23C 4/067** (2016.01)  
**B22F 1/16** (2022.01)  
**B22F 3/115** (2006.01)  
**B22F 7/04** (2006.01)

**(52) U.S. Cl.**

CPC ..... **B22F 3/115** (2013.01); **B22F 2007/042** (2013.01); **B22F 2202/13** (2013.01); **C23C 4/134** (2016.01)

**(56)****References Cited****U.S. PATENT DOCUMENTS**

- 6,022,598 A \* 2/2000 Tyson ..... C23C 14/221  
 427/166  
 8,668,962 B2 3/2014 Asmussen et al.  
 9,273,380 B2 3/2016 Shugart et al.  
 9,812,295 B1 11/2017 Stowell  
 10,464,680 B2 11/2019 Kinlen et al.  
 2007/0295701 A1\* 12/2007 Bodroghkozy ..... H05H 1/34  
 219/121.52  
 2012/0164429 A1 6/2012 Shah et al.  
 2014/0342093 A1\* 11/2014 Hadidi ..... H05H 1/30  
 264/15  
 2016/0059535 A1 3/2016 Koba et al.  
 2016/0136928 A1 5/2016 Zhao et al.  
 2017/0298476 A1 10/2017 Braydich et al.  
 2018/0073110 A1 3/2018 Balachandran et al.  
 2018/0099871 A1\* 4/2018 Tanner ..... H01J 37/32229  
 2018/0237709 A1 8/2018 Potgieter  
 2019/0256925 A1 8/2019 Braydich et al.

Baig, Z., et al., "Recent Progress on the Dispersion and the Strengthening Effect of Carbon Nanotube and Graphene-Reinforced Metal Nanocomposites: A Review", Critical Reviews in Solid State and Materials Sciences, 43(1), pp. 1-46; Jan. 2, 2018.

Bakir, M., "Novel metal-carbon nanomaterials: A review on covetics", Advanced Materials Letters, 8(9): pp. 884-890 (2017).

Basu, B., "Some fundamentals on spark plasma sintering as a processing tool to fabricate biomaterials", Internet Archive, pp. 1-44; Feb. 2017.

Forrest, D., "Approaches to High Performance Conductors", Next Generation Electric Machines Workshop, NIST, Gaithersburg, MD, Sep. 8, 2015; 64 pages.

International Search Report and Written Opinion dated May 20, 2020 for Appl. Ser. No. PCT/US2020/015133, filed Jan. 27, 2020; 13 pages.

Owrtusky, J. et al., "Obscurants for Infrared Countermeasures II", NRL/FR/6110-00-9945; Naval Research Laboratory, Washington, DC, Mar. 24, 2000; 31 pages.

Saboori, A., et al., "An Overview of Metal Matrix Nanocomposites Reinforced with Graphene Nanoplatelets: Mechanical, Electrical and Thermophysical Properties", Metals, 8(6); Jun. 5, 2018, p. 423 (33 pages).

Salamanca-Riba, L. et al., "A New Type of Carbon Nanostructure Formed Within a Metal-Matrix", Conference Paper, University of Maryland and Naval Surface Warfare Center; Jan. 2012; 6 pages. Uglov et al., Mechanical properties of copper/carbon nanocomposite films formed by microwave plasma assisted deposition techniques from argon-methane and argon-acetylene gas mixtures Apr. 2005, Composites Science and Tech., 65(5), pp. 785-791 (2005).

Wang et al., "Improvement of interfacial interaction and mechanical properties in copper matrix composites reinforced with copper coating carbon nanotubes", Jan. 2018, Materials Sci. and Engineering: A, 715, pp. 163-173.

Washington State University, "Structures of Metals", Internet Archive, pp. 1-6; Jan. 2017.

\* cited by examiner



FIG. 1A



FIG. 1B



FIG. 2



FIG. 3



FIG. 4





FIG. 6



FIG. 7

\* Robust materials interfacing and bulk deposited materials synthesis and coatings



FIG. 8A



FIG. 8B



*FIG. 9*



FIG. 10



FIG. 11  
(PRIOR ART)



FIG. 12



FIG. 13  
(PRIOR ART)



FIG. 14



FIG. 15



FIG. 16



FIG. 17



FIG. 18A1



FIG. 18A2



FIG. 18B



FIG. 18C



FIG. 18D



FIG. 19





FIG. 20A2



FIG. 20B

**FIG. 21A**

Configure a microwave reactor with (1) an inlet for a process gas (2) an inlet for a metal melt, and (3) an exit port 21B02

Introduce a hydrocarbon process gas into a first region of the reactor such that the hydrocarbon process gas dissociates into carbon and hydrogen species before reaching the metal melt 21B10

Introduce a metal melt into a second region of the reactor 21B20

Maintain the temperature in the second region until the dissociated carbon mixes with the metal melt

21B30

To next page

**FIG. 21B**



**FIG. 21B cont.**



FIG. 21C

**FIG. 22A**

**FIG. 22B**

From previous page

Move the mixture into a third region of the reactor **22B40**

Reduce the temperature of the mixture until at least some of the molten metal wraps around at least some of the carbon particles

**22B50**

Move the mixture through the exit port **21B60**

Deposit the mixture onto a substrate **21B70**

*FIG. 22B cont.*



**FIG. 23A**



**FIG. 23B**



**FIG. 23C**



**FIG. 23D**



**FIG. 24A**



**FIG. 24B**



**FIG. 25A**



**FIG. 25B**







FIG. 26E

**FIG. 27A**



FIG. 27B1





FIG. 27C

**FIG. 28**

From previous page

Introduce the melted selected powdered covetic material into a mold  
**2840**

Maintain a prescribed temperature and a prescribed pressure inside  
the mold for a prescribed duration **2850**

Bring the temperature and pressure inside the mold to about 30  
degrees C and about atmospheric pressure **2860**

Remove the mold to release the component **2870**

Deploy the component in the  
application **2880**

***FIG. 28 cont.***



FIG. 29

## 1

**APPARATUSES AND METHODS FOR  
PRODUCING COVETIC MATERIALS USING  
MICROWAVE REACTORS**

**RELATED APPLICATIONS**

This patent application is a divisional application of U.S. patent application Ser. No. 16/752,693 entitled "COVETIC MATERIALS" and filed on Jan. 27, 2020, which is a continuation in part of U.S. patent application Ser. No. 16/460,177 entitled "PLASMA SPRAY SYSTEMS AND METHODS" and filed on Jul. 2, 2019, which claims priority to U.S. Provisional Patent Application No. 62/720,677 entitled "PLASMA SPRAY SYSTEMS AND METHODS" and filed on Aug. 21, 2018, to U.S. Provisional Patent Application No. 62/714,030 entitled "PLASMA SPRAY DEPOSITION" and filed on Aug. 2, 2018, to U.S. Provisional Patent Application No. 62/903,649 filed on Sep. 20, 2019, to U.S. Provisional Patent Application No. 62/868,493 filed on Jun. 28, 2019, to U.S. Provisional Patent Application No. 62/839,995 filed on Apr. 29, 2019, and to U.S. Provisional Patent Application No. 62/797,306 filed on Jan. 27, 2019. The disclosures of all prior applications are considered part of and are incorporated by reference in this patent application.

**TECHNICAL FIELD**

This disclosure generally relates to making and using covetic materials.

**BACKGROUND**

The term covetic materials refers to metals infused with nanoscale-sized carbon particles. Covetic materials are desired in various applications since covetic materials possess many physical, chemical, and electrical properties that exceed the capabilities of traditional non-carbon infused materials. Moreover, covetic materials that derive from conventional covetic material generation techniques fail to achieve many of the aforementioned physical, chemical, and electrical properties.

Even in the face of strong demand for materials that exhibit the aforementioned physical, chemical, and electrical properties, many technical challenges have impeded development of techniques for making and using covetic materials. These technical challenges have arisen in multiple areas, including: (1) difficulties in combining analytical methods needed to measure carbon content and the characterization of the micro- or nano-structures of individual compounds with a high degree of specificity; (2) relatively high variability of carbon content distribution in samples produced thus far; (3) variability and potential unpredictability in property measurements; (4) uncertainties concerning the exact scientific mechanisms responsible for the observed strong bonding between carbon particles and their surrounding matrix.

Conventional metal melting methods used to produce covetic carbon-metal composite alloys suffer from inconsistent conversion yields, contributing to the observed wide variations in resultant material properties. For instance, unwanted formation of agglomerates and unwanted clustering often occurs due to irregularities in dispersion of carbon in the melt. Such irregularities in dispersion of carbon in the metal can lead to formation of cracks and pores that ultimately cause premature failure of the resultant material. Further, the high solubility of carbon in a metal may result

## 2

in non-uniform (such as thicker) carbon growth at the surface of the metal as the metal cools and solidifies. Additionally, solubility of carbon may be higher near a free surface than in the bulk of the metal, where higher solubility combined with interfacial energy at the melt-air interface favors undesirable precipitation at the melt-air interface.

Conventional thermal-based metal melting methods to produce covetic carbon-metal composite alloys currently cannot facilitate tuning of process conditions such that the 10 resultant covetic materials exhibit a set of desirable tuned or target properties. An inability to control process conditions such that the resultant covetic materials exhibit a set of tuned properties leads to (a corresponding) an inability to apply covetic materials to specific uses that demand such specific 15 sets of properties. What is needed are techniques to produce resultant covetic materials that exhibit a range of tunable properties. Furthermore, what is needed are resultant covetic materials that can be used in wide range of end-use areas and applications (such as business-to-business or consumer 20 uses, ranging from material strengthening to longevity performance enhancements, etc.)

**SUMMARY**

25 This Summary is provided to introduce in a simplified form a selection of concepts that are further described below in the Detailed Description. This Summary is not intended to identify key features or essential features of the claimed subject matter, nor is it intended to limit the scope of the 30 claimed subject matter. Moreover, the systems, methods and devices of this disclosure each have several innovative aspects, no single one of which is solely responsible for the desirable attributes disclosed herein.

Various implementations of the subject matter disclosed 35 herein relate generally to apparatuses, methods and various compositions of carbon-metal composite materials. The apparatuses are shown and discussed as may be relevant to controlled usage of a plasma spray torch apparatus to produce various carbon-metal bonded compositions of matter, referred to generally and in the present disclosure as "covetic materials".

One configuration of a plasma spray torch is embodied as 45 apparatus having a reaction chamber configured to receive a hydrocarbon process gas that is mixed with a plurality of molten metal nanoscale-sized particles, a microwave energy source operatively coupled to the reaction chamber to provide power thereto, and a controller to adjust the microwave energy source to create conditions in the reaction chamber such that the hydrocarbon process gas dissociates into its 50 constituent carbon atoms, and single layer graphene (SLG) or few layer graphene (FLG) is grown from the carbon atoms onto the molten metal nanoscale-sized particles to form a plurality of carbon-metal nanoscale-sized particles. In some configurations, the conditions in the reaction chamber cause: (i) a first temperature at which the carbon atoms 55 dissolve into the molten metal nanoscale-sized particles, and (ii) a second temperature at which at least some of the dissolved carbon atoms combine with the molten metal in a crystallographic configuration. Some configurations of the apparatus avail of a cooling zone to cool the plurality of carbon-metal nanoscale-sized particles to a powdered form that can be collected and stored in a containment vessel that is juxtaposed in proximity with the reaction chamber.

60 Details of one or more implementations of the subject matter described in this disclosure are set forth in the accompanying drawings and the description below. Other features, aspects, and advantages will become apparent from

the description, the drawings and the claims. Note that the relative dimensions of the following figures may not be drawn to scale.

#### BRIEF DESCRIPTION OF THE DRAWINGS

Implementations of the subject matter disclosed herein are illustrated by way of example and are not intended to be limited by the figures of the accompanying drawings. Like numbers reference like elements throughout the drawings and specification. Note that the relative dimensions of the following figures may not be drawn to scale.

FIG. 1A is a comparison chart showing two different covetic material formation techniques and example materials that result from application of each, respectively, according to some implementations.

FIG. 1B presents a high-resolution transmission electron microscopy image and a high-resolution energy dispersive spectroscopy x-ray image, according to some implementations.

FIG. 2 depicts a manufacturing process for growing graphene onto small molten particles, in accordance with one or more of the disclosed implementations.

FIG. 3 depicts a plasma energy state chart showing how a pulsed microwave energy source is used for growing graphene onto small molten particles, in accordance with one or more of the disclosed implementations.

FIG. 4 depicts an electron temperature control technique that is used for growing graphene onto small molten particles, in accordance with one or more of the disclosed implementations.

FIG. 5 illustrates a dual plasma torch apparatus that is used for growing graphene onto small molten particles, in accordance with one or more of the disclosed implementations.

FIG. 6 illustrates a pulsed microwave plasma spray torch apparatus that is tuned for growing graphene onto small molten particles, in accordance with one or more of the disclosed implementations.

FIG. 7 is a diagram depicting the intersection of common subject matter areas associated with covetics (or related materials), plasma torch spraying, and/or robust synthesized complex carbon coatings, in accordance with one or more of the disclosed implementations.

FIGS. 8A-B are schematics depicting plasma spray processes that are used for spraying carbon particles onto small molten particles, in accordance with one or more of the disclosed implementations.

FIG. 9 is a scanning electron microscope image showing the effect of spraying carbon particles onto small molten particles, in accordance with one or more of the disclosed implementations.

FIG. 10 shows a chart depicting a graphene growth temperature profile and a binary phase diagram, in accordance with one or more of the disclosed implementations.

FIG. 11 is a cross-section view of a plasma flame apparatus, in accordance with one or more of the disclosed implementations.

FIG. 12 depicts a pulsed microwave process flow that is used when growing graphene onto small molten particles, in accordance with one or more of the disclosed implementations.

FIG. 13 is a perspective view of a pulsed microwave plasma spray waveguide apparatus that is used for growing graphene onto small molten particles, in accordance with one or more of the disclosed implementations.

FIG. 14 is a schematic depiction of a micro-welding technique that is used for growing graphene onto small molten particles, in accordance with one or more of the disclosed implementations.

FIG. 15 is a schematic depiction of a plasma spray apparatus in a coaxial configuration, in accordance with one or more of the disclosed implementations.

FIG. 16 is a schematic depiction of a plasma spray apparatus showing the evolution of materials by processing 10 through a series of non-equilibrium energy conditions, in accordance with one or more of the disclosed implementations.

FIG. 17 depicts a surface wave plasma system for growing graphene onto molten particles, in accordance with one 15 or more of the disclosed implementations.

FIG. 18A1-2, FIG. 18B, FIG. 18C, and FIG. 18D depict various configurations of a plasma spray reactor, in accordance with one or more of the disclosed implementations.

FIG. 19 is a chart that depicts energy versus time during 20 pulse on and pulse off, in accordance with one or more of the disclosed implementations.

FIG. 20A1 are images depicting organo-metallic bonding that occurs when combining carbon and copper using a plasma spray torch, in accordance with some of the disclosed 25 implementations.

FIG. 20A2 are images depicting a graded composition of matter applied into a substrate material and showing multiple (such as three) material property zones, in accordance with some of the disclosed implementations.

FIG. 20B is a materials evolution chart depicting several 30 layered configurations that occur when adding carbon to bulk aluminum, in accordance with one or more of the disclosed implementations.

FIG. 21A depicts an apparatus for spraying a molten 35 mixture of materials into a substrate, according to an implementation.

FIG. 21B depicts a method for spraying covetic materials into a substrate, in accordance with one or more of the disclosed implementations.

FIG. 21C is a schematic depicting a plasma spray process 40 that is used for spraying a film, in accordance with one or more of the disclosed implementations.

FIG. 22A depicts an apparatus for wrapping carbon particles with a molten metal, in accordance with one or more 45 of the disclosed implementations.

FIG. 22B depicts a method for wrapping carbon particles with a molten metal, in accordance with one or more of the disclosed implementations.

FIG. 23A, FIG. 23B, FIG. 23C, and FIG. 23D, depict 50 example deposition techniques, in accordance with one or more of the disclosed implementations.

FIG. 24A and FIG. 24B depict conventional deposition techniques for placing materials onto a substrate, in accordance with one or more of the disclosed implementations.

FIG. 25A and FIG. 25B depict example deposition techniques 55 that result in covalent bonding at the surface of a substrate, in accordance with one or more of the disclosed implementations.

FIG. 26A, FIG. 26B, FIG. 26C, FIG. 26D, and FIG. 26E 60 depict schematic diagrams that illustrate how covalent bonds are formed between sites in the square shapes of a face-centered cubic structure of aluminum and sites in the hexagonal shapes that occur in certain crystallographic structures of carbons.

FIG. 27A depicts an example apparatus for producing 65 covetic material in a powdered form, in accordance with one or more of the disclosed implementations.

FIG. 27B1 and FIG. 27B2 depict an example fluidized bed apparatus for cooling and handling powdered covetic materials in a fluid, in accordance with one or more of the disclosed implementations.

FIG. 27C is a schematic depicting a plasma spray process that is used for production of a powdered covetic material, in accordance with one or more of the disclosed implementations.

FIG. 28 depicts method for making components from powdered covetic materials using injection molding techniques, according to some implementations.

FIG. 29 depicts various properties of covetic materials.

attributed to formation of strong interfaces that promote efficient strengthening mechanisms. Enhancements in tensile and yield strength were reported for nanosized particles (~20 nm) versus micron sized particles (~3.5  $\mu\text{m}$ ), although with as much as an order of magnitude less volume loading of the nano-size particles versus the micron-sized particles. Legacy techniques may thus fail to provide reinforcement at nanometer scales. Accordingly, there is a current need for the reduction of carbon structures having interstitial vacancies contained therein down to the nanometer scale.

#### Microwave (MW) Plasma Torch Reactor

Using a microwave (MW) plasma torch reactor, pristine 3D few layer graphene (FLG) particles can be continuously nucleated, such as in-flight in an atmospheric-pressure vapor flow stream of a carbon-containing species, such as methane gas, where such nucleation occurs from an initially synthesized carbon-based or carbon-including “seed” particle. Ornate, highly structured and tunable 3D mesoporous carbon-based particles composed of multiple layers of FLG (such as 5-15 layers) are grown from the carbon-containing species along with concomitant incorporation of metal elements or metal-based alloys to form at least partially covalently bonded (as well as at least partially metallically or ionically bonded) carbon-metal composite, also referred to herein as “covetic”, particle structures. In some implementations, “pristine” graphene (referring to graphene with no defects, or very few defects) is provided or generated in the described MW torch reactor is not oxidized, or contains very little (such as <1%) oxygen content. By itself, in some implementations, metal (in the resultant covetic materials) is held together by metallic bonding and, by itself, carbon (prevalent in graphene or some other organized carbon based 2D or 3D structure, such as a matrix or lattice), is held together by (primarily) covalent bonds. The composite carbon-metal structure may include covalent bonds between the carbon and metal atoms that occur at the metal-carbon interface.

Presently disclosed microwave plasma-based reactor processes provide a reaction and processing environment in which gas-solid reactions can be controlled under non-equilibrium conditions (referring to physical systems that are not in thermodynamic equilibrium but can be described in terms of variables that represent an extrapolation of the variables used to specify the system in thermodynamic equilibrium; non-equilibrium thermodynamics is concerned with transport processes and with the rates of chemical reactions, and the incipient melting of metal powders that can be independently controlled by ionization potentials and momentum along with thermal energy). After nucleation in-situ (referring to in-place within the reactor or reaction chamber), exiting solid, substantially solid, or semi-solid carbon-based particles from the plasma torch can be deposited in an additive, layer-by-layer fashion onto a temperature-controlled substrate (such as a drum). The exiting particles can be sprayed onto and bonded onto or into a specific substrate. In some instances, a substrate is not used, rather, groupings of exiting semi-solid particles form one or more directionally organized, free-standing, self-supported structures. Unlike a standard plasma torch where operational flows, power and configuration are limited, presently disclosed microwave plasma torch includes control mechanisms (such as flow control, power control, temperature control, etc.) to independently control one or more constituent material temperatures and gas-solid reaction chemistries to create unique, ornate, highly-organized, covalently-bound carbon-metal structures having a favorably surprising and extremely high degree of homogeneity.

#### DETAILED DESCRIPTION

Aspects of the present disclosure are directed to approaches for creating covetic materials using spraying techniques, rather than by mixing carbon-based materials into the bulk of a molten metal slurry. Some implementations relate to techniques for reduction of the size of interstitial carbon structures down to the nanometer (nm) scale. The accompanying figures and discussions herein present example environments, example systems, and example methods for creating “covetic” materials, understood generally and defined herein to imply comprised of high concentrations (>6% wt) of carbon, integrated into metals (or metal-containing materials) in such a way that the carbon does not separate out during melting or magnetron sputtering. The resulting material has many unique and improved properties over the base metal from which it is produced. The carbon is dispersed through the metal matrix in several ways that contribute to improvements in material properties. The carbon is bound into covetic material very strongly, often resisting many standard methods at detecting and characterizing its form. Inclusion of nanoscale carbon raises the melting points and surface tension. Covetics have higher warm-worked and cold-worked strengths.

#### Identification and Significance of Problem and Opportunity

Metal matrix composites may be composed of (at least) a metal or metal alloy (referring to a metal made by combining two or more metallic elements, especially to give greater strength or resistance to corrosion) matrix, in combination with a higher strength modulus ceramic, carbon-based reinforcement, or micro filler in the form of continuous or discontinuous fibers, whiskers, or particles. The size of the reinforcement is important as micron-sized reinforcement metals may exhibit improved strength and stiffness up to acceptable levels over base alloys. Nevertheless, such improvements may also be accompanied with undesirably poor ductility and undesirably low yield strength, machinability, and fracture toughness at threshold loadings due to undesirable agglomeration between particles during processing. To avoid premature cracking and other shortcomings of metal matrix composites with incompatible micron-sized reinforcements, it can be essential to reduce the size of a reinforcing phase to nanometer scale. Further, methods are needed such that the reinforcing phase is incorporated into the metal alloy matrix.

Significant increases in mechanical, thermal, electrical, and tribological (referring to the science and engineering of interacting surfaces in relative motion) properties have been observed commensurate with the addition of the aforementioned carbon-based reinforcement. Notably, such properties may change and/or improve as the size of the reinforcement is reduced from a micron scale to a nanoscale (such as <100 nm) due to increased cohesion forces between the matrix and the particles. The improvement in properties can be

Covetic materials produced by the presently disclosed MW reactor-based techniques yield various competitive advantages otherwise not available in current materials or products. One such advantage relates to an inherent scalability and versatility to formulate unique, physically and chemically stable, versatile metal-carbon composites exhibiting predictable deformation (referring to stress, strain, elasticity, or some other ascertainable physical characteristic) in a variety of configurations and/or architectures such as (but not limited to): (1) dense thin film implantations, (2) coatings, (3) thick strips, and (4) powdered particles that can be subjected to subsequent re-melting and casting and/or for use in forming engineered metal alloy components. Any of the foregoing dense thin film MW-reactor produced carbon-based metal composite implantations and/or coatings, and/or strips, and/or powdered particles all exhibit enhanced physical, chemical, and electrical properties as compared with existing parent metal alloy formulations.

#### Overview

The disclosure herein describes integration of a low dose nanofiller carbon-based material such as graphene, known for its inherent structural characteristics such as a high aspect ratio and "2D" planar geometry, with metals. Graphene possesses astonishing favorable mechanical, physical, thermal and electrical properties due to its in-plane  $sp^2$  C=C bonding (resulting in 2D planar geometry). Therefore, graphene would serve as an ideal reinforcement for metal matrix composites as compared with alternatives such as micro-filler polyacrylonitrile (PAN)-based carbon fiber. It should be noted that even at low graphene nanoplatelet content (loadings), a 3D network is formed with an anisotropic (referring to an object or substance having a physical property that has a different value when measured in different directions), that result in marked improvements to thermal and electrical conductivities as well as mechanical features.

A challenge encountered in using carbon nanofillers in metal matrix composites includes difficulty with dispersion due to poor wetting (referring to the ability of a liquid to maintain contact with a solid surface, resulting from intermolecular interactions when the two are brought together; the degree of wetting, referred to as wettability, is determined by a force balance between adhesive and cohesive forces). The increased surface area presented by nanofillers causes particles to agglomerate into clusters and twists due to Van der Waals forces between carbon atoms. Agglomerates and clustering of nanofillers in metal matrix composites can lead to formation of undesirable cracks and pores that may ultimately compromise structural integrity of the resultant material yielding premature failure under high load or performance conditions.

Although a number of processing approaches, such as conventional powder metallurgy, hot rolling, casting, and additive manufacturing have been (and may currently also be) used to produce metal matrix composites, there are still challenges with uniformly dispersing nanofillers. Damage to nanofiller from applied stress during consolidation, and undesirable or uncontrollable chemical reactions with the matrix at elevated temperatures during sintering and casting, are some examples of challenges faced during attempts to achieve nanofiller dispersion.

Defect free, the basal plane of graphene exhibits exceptionally favorable chemical stability compared to sides and ends of a graphene sheet, which may be more prone to interact with metals to form carbides (thermodynamically favored as per the Gibbs free energy). During processing, however, defects can readily form in the basal plane, leading

to carbide formation and adverse effects to composite properties. Hence, relatively severe processing conditions such as high temperatures and pressures, can adversely affect the quality of the interface between carbon nanofillers and their surrounding metal-based matrix. Specifically, high temperatures and pressures can adversely affect wetting ability, structural integrity, may unwantedly influence carbide formation, and may otherwise cause other deleterious interface reactions.

An alternative process, referred to as covetics (as introduced earlier), has been successfully used to incorporate carbon nanofillers into metal matrices. In covetic related processes, a network of graphene 'ribbons' and nanoparticles have been shown to form within a liquid metal by using an applied electric field that exhibits exceptional stability within the metal matrix, even after re-melting. Correspondingly, the composite structure conducts heat and electricity more efficiently than the parent metal.

#### Uniform Dispersion

Since one of the challenges to incorporating graphene into a metal matrix is achieving uniform dispersion, covetics processing overcomes this problem through the concomitant exfoliation and wetting of the graphene ribbons and/or particles within an applied electric field (either from the carbon electrodes or from the breakdown of carbon additives). Impurities, such as oxygen and hydrogen, can be managed via redox reactions at the particle surface, assuming a properly induced voltage at the surface, to promote wetting/dispersion. A challenge is one of controlling the structural integrity and uniformity of the graphene ribbons and/or particles (such as uniformity with respect to size, defects, etc.), as well as controlling chemical reactivity with the metal at elevated temperatures, and as well as controlling distribution of particles in the bulk as well as at the surface of the melt.

#### Additional Complexities

Although fundamental modes of energy conduction in metals (both thermal and electrical) can be (at least in part) carried out by electrons and is controlled by the degree of crystallinity and impurities for a filler such as graphene to enhance thermal conductivity in the metal matrix composite (where conduction is via phonons in graphene), there either needs to be some degree of registry and/or coherency (such as an integrally bound nano scale carbon) with the metal lattice (additionally or alternatively referred to as a scaffold, matrix, or structure) or a minimum platelet spacing (such as proximity or network) threshold for conduction between platelets (such as the graphene would need to be a single layer or just a few layers and 10's of nanometers in length). With respect to strengthening the metal matrix, however, graphene may need to be chemically (or in some instances, also physically) bonded to the matrix for proper load transfer (noting that the length of graphene can be greater than ~0.5  $\mu\text{m}$  for maximum load transfer). Aside from solid solution strengthening, which relies on coherent and/or semi-coherent elastic strains between carbon (graphene) nanofiller and metal lattice, a discrete graphene nanoparticle can serve as a barrier to dislocation pile-up or pinning (such as Hall Petch grain refinement, referring to a method of strengthening materials by changing their average crystallite (grain) size; it is based on the observation that grain boundaries are insurmountable borders for dislocations and that the number of dislocations within a grain have an effect on how stress builds up in the adjacent grain, which will eventually activate dislocation sources and thus enabling deformation in the neighboring grain, too; so, by changing grain size one can influence the number of dislocations piled up at the grain

boundary and yield strength) at grain boundaries, both of which improve mechanical properties.

Again, because of its 2D nature and high surface area, graphene can orient along regions at grain boundaries in addition to aligning along slip planes within the metal structure. Irrespective of whether the property of interest is chemical, mechanical, thermal or electrical, the greater the alignment and registry of the nanofiller to the crystal structure of the surrounding metal matrix (at the atomic level), the greater the enhancement as well as stability of the property in a metal matrix composite structure.

Fundamentally, growth of carbon at a metal surface (heterogeneous) or precipitation out of solution in the melt (homogeneous) is dependent on the solubility of carbon in the metal (as per the binary phase diagram shown on the right side of FIG. 10). The solubility of carbon in pure transition metals (and many pure metals, generally) is very low, such as near the melting point of the metal, although increases as the temperature increases to well above the melting point of the metal (such as up to 2,000° C. and above). The solubility of carbon in nickel, for example, near the hypereutectic point of around 2.5% is one of the higher solubilities of carbon in a pure metal. Note that the addition of interstitial impurities such as oxygen, boron, or nitrogen, or substitutional atoms to a metal, can affect (such as potentially increase) the solubility of carbon. It has been shown that the higher the solubility of carbon in a metal, or the higher the temperature of the molten metal, the thicker the carbon that precipitates at the surface of the metal as the metal is cooled down and solidified. Important to note is that solubility of carbon is higher near a free surface, which, in combination with the interfacial energy of the liquid-air interface, favors precipitation of solid carbon at the metal melt-air interface. Equipment and techniques for operating the equipment to overcome the problems attendant to this phenomenon are addressed as pertains to the figures and corresponding discussions.

#### Definitions and Use of Figures

Some of the terms used in this description are defined below for easy reference. The presented terms and their respective definitions are not rigidly restricted to these definitions—a term may be further defined by the term's use within this disclosure. The term “exemplary” is used herein to mean serving as an example, instance, or illustration. Any aspect or design described herein as “exemplary” is not necessarily to be construed as preferred or advantageous over other aspects or designs. Rather, use of the word exemplary is intended to present concepts in a concrete fashion. As used in this application and the appended claims, the term “or” is intended to mean an inclusive “or” rather than an exclusive “or”. That is, unless specified otherwise, or is clear from the context, “X employs A or B” is intended to mean any of the natural inclusive permutations. That is, if X employs A, X employs B, or X employs both A and B, then “X employs A or B” is satisfied under any of the foregoing instances. As used herein, at least one of A or B means at least one of A, or at least one of B, or at least one of both A and B. In other words, this phrase is disjunctive. The articles “a” and “an” as used in this application and the appended claims should generally be construed to mean “one or more” unless specified otherwise or is clear from the context to be directed to a singular form.

Various implementations are described herein with reference to the figures. It should be noted that the figures are not necessarily drawn to scale, and that elements of similar structures or functions are sometimes represented by like reference characters throughout the figures. It should also be

noted that the figures are only intended to facilitate the description of the disclosed implementations—they are not representative of an exhaustive treatment of all possible implementations, and they are not intended to impute any limitation as to the scope of the claims. In addition, an illustrated implementation need not portray all aspects or advantages of usage in any particular environment.

An aspect or an advantage described in conjunction with a particular implementation is not necessarily limited to that implementation and can be practiced in any other implementations even if not so illustrated. References throughout this specification to “some implementations” or “other implementations” refer to a particular feature, structure, material or characteristic described in connection with the implementations as being included in at least one implementation. Thus, the appearance of the phrases “in some implementations” or “in other implementations” in various places throughout this specification are not necessarily referring to the same implementation or implementations. The disclosed implementations are not intended to be limiting of the claims.

#### DESCRIPTIONS OF EXAMPLE IMPLEMENTATIONS

FIG. 1A is a comparison chart 1A00 showing two different covetic material formation techniques 102 and example materials that result from the application of each, respectively.

In the case of conventional metal melt methods 103 to produce covetic materials, solid carbon is added to a metal melt. This conventional metal melt technique is governed by the kinetics of carbide formation and interdiffusion across a solid-liquid (such as carbon-metal) interface under an applied current, which provides additional energy to overcome stacking fault energy between carbon atoms and metal atoms. As such, conventional metal melt techniques for forming covetic processing do not significantly differ from other composite processing methods, such as powder metallurgy and/or hot rolling, which composite processes involve consolidation of a second phase particle into a metal matrix. These conventional composite processing methods face many challenges with dispersion and/or distribution, reactivity, and variability in material properties. Furthermore, conventional covetic processing relies on batch processing, and often yields inconsistent conversion yields as well as wide variations in resultant properties.

As depicted by agglomeration image 105, when using conventional metal melt methods 103, the resultant material suffers from extreme agglomeration of carbon, which in turn: (1) limits the role of carbon to reinforce the lattice; and, (2) limits the tunability of the surface morphology for surface functionalization. For comparison, when using presently disclosed techniques, the resultant material exhibits nearly uniform homogeneity (such as no agglomerates), which homogeneity results from uniform dispersion of carbon into the lattice. This is shown in homogeneity image 106.

Covetic materials such as are depicted in homogeneity image 106 can be characterized by many desirable material properties 108 such as uniformity, high carbon loading, low carbon content at surfaces, etc. These are highly desirable material properties that are not exhibited by materials formed using conventional metal melt methods 103. Therefore, what is sought after are improved approaches that overcome shortcomings of the conventional metal melt methods 103.

One such improved approach involves plasma spray torch methods 104. Application of plasma spray torch methods result in a consistent yield of covetic materials, thus overcoming the yield shortcomings of conventional metal melt methods. Furthermore, application of plasma spray torch methods results in covetic materials that possess the aforementioned improved mechanical, improved thermal, and improved electrical properties, thus overcoming resultant material shortcomings of conventional metal melt methods.

#### Improved Approaches

As shown, the plasma spray torch methods 104 can be configured to use input materials as introduced (referring to provision of a carbon-containing feedstock species in gaseous form, such as methane, and energizing it via application of MW energy directed through the methane gas, etc.). However, by dissociating carbon-containing gas (such as methane or other hydrocarbon sources) at elevated temperatures, a self-limited monolayer of carbon—and in particular, pristine graphene—can be grown onto and/or into a metal (such as copper, gold, zinc, tin, and lead) lattice. The number of monolayers is dependent at least in part on the solubility of carbon in the metal. Growth kinetics, binding, and the final structure of graphene films onto a metal substrate is dependent on the valence electrons and the symmetry (close packed planes) of the metal. Similarly, metals can be grown on carbon, preferentially nucleating and growing at defect sites of the carbon or at selective oxygen- or hydrogen-terminated sites as well. Alternating stacks of single layer carbon and metal can then be fabricated to realize the enhanced properties of a graphene-reinforced metal composite structure.

Using a microwave plasma reactor, pristine 3D few-layer graphene particles can be continuously nucleated and grown from a hydrocarbon gas source. In addition, selective elements can be incorporated into the 3D graphene particle scaffold by adding them to the plasma gas stream. The microwave plasma reactor process provides a unique reaction environment in which gas-solid reactions can be controlled under non-equilibrium conditions (such as chemical reactions can be independently controlled by ionization potentials and momentum along with thermal energy). Reactants can be inserted as solids, liquids or gases into a plasma reactor zone to independently control nucleation and growth kinetics of unique non-equilibrium structures (such as graphene on metal and metal on graphene).

For example, to create integrated graphene-metal composites at the nanometer scale, fine nanometer-scale metal particles can be introduced into a microwave plasma torch along with a hydrocarbon gas such as methane. Methane dissociates into hydrogen and carbon (such as using the ideal energy of the microwave plasma to form C and  $C_2$ ) which can then nucleate and grow ordered graphene onto the semi-molten surface of the metal particle. Non-equilibrium energy conditions can be created by tuning process conditions to independently control the temperature of the metal with respect to carbon reactivity and delivery to the metal surface. Ionized hydrogen (or other ions) at controlled low energies can be used to impinge/sputter the surface of the growing graphene-metal surface without damaging the structure of the graphene-metal composition. This then promotes further growth of alternating graphene-metal layers. In addition, depending on residence time and the energetics within the plasma reaction zone, metal-graphene structures can be created with specific properties that are retained when the metal-graphene structures are rapidly cooled upon being sprayed onto a substrate at a controlled temperature. The formation of the metal-graphene structures

at controlled energies within the plasma as well as control of the temperature of the substrate provides independent control of energetic conditions throughout the entire evolution of these covetic materials.

Graphene can be applied (and/or deposited) onto metal or metal-containing layers of material via “sputtering” (referring to a phenomenon in which microscopic particles of a solid material are ejected from its surface, after the material is itself bombarded by energetic particles of a plasma or gas; the fact that sputtering can be made to act on extremely fine layers of material is often exploited in science and industry—there, it is used to perform precise etching, carry out analytical techniques, and deposit thin film layers in the manufacture of optical coatings, semiconductor devices and nanotechnology products, etc.). Such sputtering, as so described, can be controlled by controlling residence times and energetics within the plasma reaction zone to promote growth of alternating graphene-metal layers when employed with the presently discussed MW plasma reactors. These alternating graphene-metal layers are organized in coherent planes of atoms that are in a regular (such as crystallographic) configuration. This crystallographic configuration is retained when the graphene-metal layers are quickly quenched (in the materials science field, quenching, or quick/rapid quenching, refers to the controlled rapid cooling of a workpiece in water, oil or air to obtain certain material properties; a type of heat treating, quenching prevents or controls undesired low-temperature processes, such as phase transformations, from occurring by reducing the window of time during which these undesired reactions are both thermodynamically favorable and kinetically accessible; for instance, quenching can reduce the crystal grain size of both metallic and plastic materials, increasing their hardness) onto a cooler substrate. Quick quenching, as so described, serves to essentially ‘freeze’ (referring to retention in a substantially solid state rather than solely on the traditional definition of change in phase from a liquid to a solid) graphene to metal in a desired crystallographic configuration formed within the plasma reactor. The homogeneity within and at the surface of the resultant material is extremely uniform. This extremely uniform homogeneity can be used to distinguish from materials that had been formed using metal melt methods 104. This is because the metal melt methods 104 cannot control ion energies independently from thermal energies. More specifically, because the metal melt methods 104 cannot achieve the desired higher ion energies independently from thermal energies, temperatures in the metal melt reaction chamber can be too high for graphene-metal layers to become organized in coherent planes of atoms that are in the desired crystallographic configuration.

Therefore, when using metal melt methods 104, the desired crystallographic configuration of the graphene-metal never occurs, and thus desired crystallographic configuration cannot be retained when the graphene-metal layers are quenched onto a cooler substrate. Instead, when using metal melt methods 104, undesired carbon precipitation occurs (such as carbon precipitates out of the melt), which in turn leads to unwanted agglomeration, which in turn leads to non-uniformity in the resultant. This non-uniformity in the resultant can lead to less than ideal chemical and/or physical (mechanical) characteristics in the resultant materials, including but not limited to premature mechanical failure.

FIG. 1B presents a high-resolution transmission electron microscopy image 114 and a high-resolution energy dispersive spectroscopy x-ray image 116. Also shown here for convenience is the homogeneity image 106 of FIG. 1A.

As depicted by this example set of images, the carbon is distributed uniformly throughout the metal lattice. This is emphasized in the high-resolution transmission electron microscopy image 114. Moreover, the extremely high carbon loading in the metal lattice is clearly shown by the high-resolution energy dispersive spectroscopy x-ray image 116. In this example, the carbon loading forms approximately 60% of the overall copper-carbon lattice. This is shown in the high-resolution energy dispersive spectroscopy x-ray image 116. In this particular image, the darker areas are carbon and the lighter areas (appearing as dots) are copper.

As can be seen the images, and in particular, as can be seen from the pattern of the high-resolution energy dispersive spectroscopy x-ray image 116, the carbon and the parent metal (such as in this case copper), are uniformly dispersed. This uniform lattice-level dispersion is present at the surface, as shown, moreover, this uniform lattice-level dispersion is also present deep into the parent metal. Additional images of covetic materials are given in FIG. 20A1, FIG. 20A2 and FIG. 20B, which figures follow after discussion of (1) materials evolution processes, (2) a plasma spray torch apparatus and (3) various configurations of plasma spray torches.

In one use scenario, the covetic materials of FIG. 1B can be manufactured using a tunable microwave plasma torch that produces integrated graphene-metal composite films at high rates and volumes. One particular manufacturing process during which graphene is grown onto small molten metal particles is now briefly discussed.

FIG. 2 depicts a manufacturing process 200 for growing graphene onto small molten particles. As an option, one or more variations of manufacturing process 200 or any aspect thereof may be implemented in the context of the architecture and functionality of the implementations described herein. The manufacturing process 200 or any aspect thereof may be implemented in any environment.

One possible method is to use a “non-equilibrium energy” microwave plasma torch to provide non-equilibrium control over the temperature of the metal independently from carbon creation. This plasma torch energy is then directed to the molten and/or semi-molten metal particles surfaces. This technique allows time for growth to occur on the melt. Growth on the melt (or semi-melt or core shell materials) created within the torch will flow out through the main plasma plume to the surface of the metal to be grown upon, and then is quickly quenched. This technique provides a means to grow thick films which, upon layering, could be grown into a homogeneous thick ingot and/or grown into or onto component parts to be post machined or remelted into applications.

Additionally, FIG. 2 is being presented to illustrate the effects that independent control of constituent material temperatures and gas-solid reaction chemistries when growing graphene onto small molten particles. FIG. 2 shows the evolution through several processes of covetic materials manufacturing; and, presents processes used in the formation of plasma torch-based covetic materials.

As shown, semi-solid particles exiting from the plasma torch can be deposited in an additive, layer-by-layer fashion onto a temperature-controlled substrate. Unlike a standard plasma torch where operational flows, as well as control of power and other configurations are limited, the discussed microwave plasma torch can be operated to independently control constituent material temperatures as well as gas-solid reaction chemistries.

As can be seen from the disclosure above, microwave plasma sources can result in (for example): (1) higher plasma densities; (2) ion energies with a narrower ion energy distribution; and, (3) improved coating properties. This is due, at least in part, to the improved power coupling and (electromagnetic energy) absorption at 2.45 GHz. Pressure dependent, typical electron temperatures are of the order of 1 eV to 15 eV yielding plasma densities of  $>10^{11} \text{ cm}^{-3}$ . Such low electron temperatures are also advantageous not only in terms of controlling the plasma chemistry, but also in terms of limiting the ion energy with ion energies for Argon-based coaxial microwave plasmas that typically are in the range of 5 eV to 80 eV. As a consequence of the narrow plasma sheath formed using these high-density plasmas, collisional broadening of the ion energy distribution is prevented, thus resulting in a sharp ion energy distribution that supports fine control of certain film deposition processes. Additionally, through the usage of pulsed power into a microwave plasma, non-equilibrium energies can be formed and controlled. During application of microwave energy, power is delivered throughout a volume where plasma is to be formed, thus energy is accumulated in a stepwise collisional energy regime.

The foregoing discussion of FIG. 2 includes techniques for application of microwave energy power, which technique is disclosed in further detail as follows.

FIG. 3 depicts a plasma energy state chart 300 showing how a pulsed microwave energy source is used for growing graphene onto small molten particles.

Microwave plasma sources have the potential to achieve higher plasma densities, ion energies with a narrower ion energy distribution, and improved coating properties as a consequence of improved power coupling and absorption at 2.45 GHz. Pressure-dependent typical electron temperatures are of the order of 1 eV to 15 eV yielding plasma densities of  $>10^{11} \text{ cm}^{-3}$ . Such low electron temperatures are also advantageous not only in terms of controlling the plasma chemistry, but also in terms of limiting the ion energy with ion energies for Argon-based coaxial microwave plasmas that typically are in the range of 5 eV to 80 eV. As a consequence of the narrow plasma sheath formed using these high-density plasmas, collisional broadening of the ion energy distribution is prevented resulting in a sharp ion energy distribution, which is necessary for fine control of some film deposition processes. Additionally, through the use of pulsed power being delivered into a microwave reactor, plasma non-equilibrium energies can be formed and controlled. During application of microwave energy, power is delivered thru a volume where plasma is to be formed, thus energy is accumulated in a stepwise collisional energy regime.

Once the initial plasma forms in the vast majority of the volume, the delivery antennae where energy is at a maximum continues to increase in a highly localized fashion. Plasma density nearby decreases slightly until the plasma constricts. Further details regarding general approaches to making and using pulsed microwave energy sources are described in U.S. Pat. No. 10,332,726, issued Jun. 25, 2019, which is hereby incorporated by reference in its entirety.

FIG. 3 shows that the initial energy of the plasma is much higher in the non-equilibrium state until it constricts to a much lower stable temperature. More specifically, the plasma energy state chart depicts a transition from an initial high energy non-equilibrium state to a lower energy stable equilibrium state. Once the initial plasma forms, the delivery antennae, where energy is at a maximum, will continue to

increase in a highly localized fashion until the plasma constricts and is lost in the remaining parts of the chamber due to energy shielding.

The pulsed microwave energy source can be controlled so as to optimize electron temperatures for growing graphene onto small molten particles. This is especially effective in the case where pressures are  $>>20$  Torr. To ensure that plasma chemistry dissociation is homogeneous, and that coating of materials is homogeneous as well, the environments of the chamber must be controlled.

As is shown in FIG. 3, the energy profile indicates that the initial energy is high and, after a time, constricts to a lower level where it stays until the power is removed. The plasma extinguishes and, after restarting, follows the energy cycle again. By reducing the time between the initial plasma ignition and where it stabilizes, the plasma remains mainly in the bulk of the system where a more homogeneous dissociation of materials can occur. The reduction of the time between the initial plasma ignition and the time when it stabilizes can be accomplished by controlling the frequency and duty cycle of pulsing.

One technique for controlling electron temperatures in a pulsed microwave reactor is shown and described as pertains to FIG. 4.

FIG. 4 depicts an electron temperature control technique 400 that is used for growing graphene onto small molten particles. As an option, one or more variations of electron temperature control technique 400 or any aspect thereof may be implemented in the context of the architecture and functionality of the implementations described herein. The electron temperature control technique 400 or any aspect thereof may be implemented in any environment.

FIG. 4 illustrates aspects pertaining to growing a few layers of graphene onto molten nanoscale-sized particles rather than mixing carbons into the bulk of a molten slurry. Specifically, the figure is being presented with respect to its contribution to controlling plasma temperature through control of microwave pulsing frequency.

#### Plasma Temperature Control Via Control of Pulsing Frequency

As depicted in the foregoing FIG. 3, the energy profile indicates that the initial energy is high and, after a time, constricts to a lower level where it stays until the power is removed. The plasma extinguishes and, after restarting, follows the energy cycle again. By reducing the time between the initial plasma ignition and stabilization, the plasma remains mainly in the bulk of the system where a more homogeneous dissociation of materials can occur.

As shown in FIG. 4, the effect depends substantially on the timing of the on/off cycle of the microwave energy source. By controlling the frequency of pulsing, optimal chemical dissociation and uniform coatings can be created. Furthermore, by setting the pulsing frequency, the average temperature of the plasma can be controlled as well.

#### Plasma Temperature Control in a Microwave Plasma Torch

The herein-discussed integrated microwave plasma torch is used for addressing the formation of integrated, second phase, carbon-metal composite structures with enhanced mechanical, thermal and electrical properties over existing metal alloys and conventional composite processing methods. Furthermore, the microwave plasma torch can be used to form carbon-metal composite coatings and particles directly onto high value asset components. Still further, the aforementioned methods and equipment meet many clean energy goals pertaining to improved electrical distribution and efficient transformer and heat exchanger performance.

#### Microwave Plasma Torch Practical Applications

Using the integrated microwave plasma torch technology, materials can be economically (such as cost effectively) deposited and/or formed at fast rates and can be applied and in a variety of different configurations. Benefactors of this technology include various energy production industries—especially as pertains to transmission and storage—transportation industries, military equipment industries, as well as many other manufacturing industries. As one specific practical application example, metallic surfaces of an aircraft can be treated by a plasma spray to create covetic material at the metal-air interface. The metallic surfaces thus become impervious to corrosion. Additionally, the carbon atoms near the surface allows for other materials to be chemically bonded to the carbon atoms and/or adhered to the surfaces. The aforementioned other materials that can be chemically bonded to the carbon atoms might be selected on the basis of requirements that arise in various practical applications.

As another specific practical application example, metallic surfaces of an airborne vehicle (such as an airplane, helicopter, drone, projectile, missile, etc.) can be treated by a plasma spray to create a covetic material coating that acts as an infrared obscurant (such as a detection countermeasure).

FIG. 5 illustrates a dual plasma torch apparatus 500 that is used for growing graphene onto small molten particles. As an option, one or more variations of dual plasma torch apparatus 500 or any aspect thereof may be implemented in the context of the architecture and functionality of the implementations described herein. The dual plasma torch apparatus 500 or any aspect thereof may be implemented in any environment.

The shown equipment setup uses: (1) a metal plasma spray torch to supply molten metals to the surface of the heated substrate (Al, Cu, Ag, etc.), and (2) a microwave plasma torch to deliver ionized carbon and plasma radicals to the molten surface so as to cause the covetics growth onto molten metals.

The system is inserted into an inert gas environment or into an atmospherically controlled chamber to provide better control of materials oxidation. In one implementation, the setup and operation of the torch of FIG. 5 is shown in Table 1, the details of which are discussed infra.

TABLE 1

| Step | Setup & Operation Description                                                                                |
|------|--------------------------------------------------------------------------------------------------------------|
| 1    | Identify and select reactant materials                                                                       |
| 2    | Integrate a standard, non-microwave plasma spray torch and a microwave plasma torch into a dual-plasma torch |
| 3    | Define plasma torch processing parameters                                                                    |
| 4    | Operate the dual plasma torch to produce graphene growth on a semi-molten particle surface                   |

#### Step D1: Reactant Material Identification and Selection

Any number of metals can be plasma-sprayed concurrently along with metastable carbon species to form a nano-carbon-metal composite structure. Different metals with high electrical and thermal conductivity can be used when forming 2D graphene at concentrations above the thermodynamic solubility limit. In some cases, two different metals are selected, each having different carbon solubility limits and/or different melting points and/or different densities and/or different crystal structures.

Step D2: Selection, Modification and Validation of Micro-wave and 'Standard' Plasma Spray Torch(es)

The apparatus of FIG. 5 can be (in certain implementations) substantially composed of a 'standard', off-the-shelf, plasma spray and a microwave plasma torch. Having two torches allows for two different processing steps, namely: (1) incipient melting of the metal, and (2) nucleation/growth of graphene platelets from a hydrocarbon source. Each one of the two torches can be controlled independently from each other.

As shown in FIG. 5, the two torches are collocated for concurrent or sequential operation. Specifically, the microwave plasma with its low electron temperature and high electron density can be used to optimize graphene formation (including nucleation rate at the carbon supersaturation threshold) whereas the standard plasma spray torch can be used to heat metal powder/particles to a molten or semi-molten state and then accelerate the particles (along with nucleated ionized carbon/graphene) towards the substrate. The two independent flow streams can be coordinated so as to accomplish fine-scale graphene growth on a semi-molten particle surface. In some cases, the dual torch configuration comprises a means to maintain an inert atmosphere (such as cover gas) at or near the exit stream of the torches and in and around the impingement region at the surface of the substrate. This is because contaminants from the surrounding air (such as oxygen, nitrogen and moisture) can affect bonding between the carbon and metal atoms. Therefore, in certain implementations, the dual torch system is configured to be inserted into a fully controlled inert gas environment (such as a chamber) so as to provide effective control of material oxidation.

Step D3: Rationale and Definition of Plasma Processing Parameters

Reactants (such as hydrocarbons) and inert gases and flows are selected to ensure the stability of plasma and to ensure control of nucleation and growth processes within the plasma (such as supersaturation thresholds for a given gas mixture and flow rate). Acceleration rates and temperatures of the metastable carbon are controlled during excursion from the plasma to the substrate. Correspondingly, process conditions for the standard plasma spray torch are set so as to create a consolidated thin film onto which carbon can impinge and react. Surface temperature and local gas phase environments are controlled so as to promote interaction and growth of the metastable carbon phase.

Step D4: Operate the Dual (Metal and Microwave) Plasma Torch

Various parameters of processing windows of both the metal and microwave plasma torch are configured to be controlled independently or, in some implementations, in conjunction with each other. Before, during and after operation of one or more of the metal and microwave plasma torches (referred to herein as "the dual plasma torch"), processing windows for integrated carbon-metal formation are characterized. Furthermore, one or more parameters or combinations of parameters are selected, deposition of carbon-metal is observed, and using any known-in-the-art techniques, the as-deposited samples can be characterized with respect to various differentiators, including (but not limited to): morphology (such as using a scanning electron microscope (SEM)), structure (such as via x-ray diffraction (XRD) and via Raman spectroscopy), and/or physical and chemical composition.

FIG. 6 illustrates a pulsed microwave plasma spray torch apparatus 600 that can be tuned for growing graphene onto small molten particles. As an example, one or more varia-

tions of pulsed microwave plasma spray torch apparatus 600 (or any aspect thereof) may be implemented in the context of the architecture and functionality of the implementations described herein. The pulsed microwave plasma spray torch apparatus 600 (or any aspect thereof) may be implemented in any environment.

In this configuration, transverse electric (TE) microwave energy power means can be coupled onto (or, in some implementations, also penetrate substantially within) a central dielectric tube to propagate microwave energy into and throughout the central dielectric tube. Gas supplied into the center region (in this example) can be a hydrocarbon gas such as methane that absorbs the microwave radiation. Metal powder is supplied (as carried by a substantially inert carrier gas) to be heated within the body (or primary chamber) of the pulsed microwave plasma spray torch apparatus 600 from the combination of the plasma-derived and applied thermal energy. Upon exposure to such energy, metal powder melts upon reaching a melting temperature to produce a viscous flowable liquid material, or droplets (potentially containing semi-solid materials), or any other conceivable dispersion (largely dependent on attendant melt conditions).

As hydrocarbon gas decomposes into its constituent element species, carbon radicals nucleate on exposed surfaces of the melted metal droplets. The combination of energy tuning settings of the microwave, and thermal plume temperature settings can allow for different temperatures between the melt temperature and the plasma decomposition/ionization temperature in a central region of the pulsed microwave plasma spray torch apparatus 600. Non-equilibrium conditions within the central chamber or region of the plasma spray torch apparatus (referring to temperature, pressure, etc.) can allow (or otherwise facilitate) internal lattice placement (referring to the positioning of a synthesized lattice structure of carbon materials with that of any input metal(s) such that individual carbon and metal atoms can be at least partially aligned) of the graphene/carbon, whereas the quick quenching creates conditions conducive to covetous materials growth. Diagrams showing internal lattices where the lattice of the carbon and the lattice of a metal are oriented such that carbon and metal atoms are at least partially aligned are presented in FIG. 8A-B, FIG. 12, FIG. 26C, and FIG. 26D and in corresponding written description, infra.

The single integrated microwave plasma torch of FIG. 6 can be set up and operated as depicted in the following Table 2, the details of which are described infra.

TABLE 2

| Step | Setup/Operation Description                                                                                      |
|------|------------------------------------------------------------------------------------------------------------------|
| 1    | Deploy a single integrated microwave plasma torch                                                                |
| 2    | Operate the single integrated microwave plasma torch for the formation of graphene-loaded metal composite alloys |
| 3    | Characterize the resultants                                                                                      |

Step S1: Deploy a Single Integrated Microwave Plasma Torch

FIG. 6 depicts a single integrated microwave plasma torch. The torch has the capability to process solid, liquid and vapor reactant feedstock species using (for example) a small inert gas or differentially pumped vacuum for controlling gas flow. The torch can be deployed in any environment (referring to laboratories, research set-ups, or large-scale industrial concerns, etc.).

Step S2: Operate the Single Integrated Microwave Plasma Torch for Formation of Graphene Loaded Metal Composite (“Covetic”) Alloys

Microwave energy is delivered in a collinear waveguide configuration along with a centralized gas feed system for efficient microwave energy absorption. The microwave energy source is used to heat the metal to a semi-molten state. As the CH<sub>4</sub> (or other hydrocarbon source) decomposes (into its constituent species) within an exhaust plume that is directed into a surface wave plasma gas dissociation tube, carbon radicals can nucleate (such as in an organized layer-by-layer manner) on the surface of the metal droplets via being energized by plasma radicals (directed onto the metal droplets). The energy tuning of the microwave thermal plume temperature and plasma allows for independent control of temperatures between the melt and the plasma decomposition/ionization that occurs within the central region of the pulsed microwave plasma spray torch apparatus 600.

Process conditions are measured and optimized. Desired process conditions are controlled by or for the integrated microwave plasma torch to directly form graphene-loaded metal composite material within a single or multi-stage plasma reaction torch. The plasma torch can be modulated within different regions of the surface wave plasma to enhance resonance (modulation) times and to optimize formation of targeted metal-carbon structures.

In addition to the shown process gas port (such as for introduction of a hydrocarbon process gas 605) at the depicted location, additional ports 604 can be provided at different locations. Such additional ports can be used to control how the process gas is introduced into the microwave field, and to introduce other process gasses. As examples, a process gas might be SiH<sub>4</sub> or NH<sub>3</sub>. In some implementations, more than one input port for gas or more than one input port for particles (such as one for carbon and one for metal) may be included, where the location of the input ports can be positioned in different zones of the plasma torch.

The foregoing setup and conditions, as well as other conditions are optimized to result in conditions at the substrate surface that enable impinging particles to be consolidated into a film. The as-deposited films are analyzed and characterized according to methods outlined in Step S3 below.

Step S3: Validate/Characterize the Graphene (Secondary Phase) Metal Properties

Characterization of the as-deposited integrated carbon-metal composite structures are accomplished using several techniques. For example, x-ray photoelectron spectroscopy (XPS) and/or SEM-EDS can be used to determine chemical composition, binding energies (nanoscale carbon detection) and distribution. Also, energy-dispersive x-ray spectroscopy (EDS) and/or SEM, and/or Raman spectroscopy, and/or XRD can be used for determining morphology and/or for measuring grain size and structural aspects. Electrical and thermal properties as well as the tensile strength and modulus of the composite material can be evaluated using any known techniques.

#### Results

The foregoing techniques use a microwave plasma torch to continuously fabricate metal matrix composites. The processing entails material nucleation and formation of a growth zone within the plasma followed by an acceleration and impaction zone for consolidation of the materials onto a substrate. Each zone provides for unique control of dissimilar materials synthesis/formulation and integration;

namely, selective and unique formulation of alloy particles within the plasma, which then, through control of momentum (primarily kinetic) and thermal energetics during impact onto a substrate, enable a unique additive process for controlling consolidation parameters such as porosity, defect density, residual stress, chemical and thermal gradients, phase transformations, and anisotropy.

Various materials are selected for use across a wide range of growth dynamics within the plasma operation environment. In particular, different hydrocarbon gas sources with specific ratios of carbon to oxygen and hydrogen, and solid metal (or metal alloy) particle sources with different carbon solubilities, melting points, and crystal structures can be processed through the pulsed energy plasma torch processing system. As such, specific plasma processing parameters can be identified for concomitant incipient surface melting of the particle along with nucleation/growth and incorporation of 2D graphene and re-sputtered metal at the metal surface.

Upon incorporation of graphene into the metal from the microwave plasma torch, as-deposited materials/films are characterized with respect to “covetic-like” properties. As examples, these covetic-like properties can be characterized as (for example): (1) chemical composition (such as to detect impurities and to detect forms of carbon); (2) distributions of carbon (such as interstitial—referring to positions of carbon atoms or species within a metal matrix or lattice, intragranular and intergranular); (3) electrical conductivity; and, (4) mechanical strength of the materials. The characterizations may include comparisons between graphene loaded versus un-alloyed parent metals. Further, and strictly as examples, using the microwave plasma torch, the as-deposited materials may exhibit a ratio of carbon to metal throughout the range (inclusive) of about 3% to 90%. In some situations, the ratio of carbon to metal is throughout the range (inclusive) of about 10% to about 40%. In some situations, the ratio of carbon to metal is throughout the range (inclusive) of about 40% to about 80%. In some situations, the ratio of carbon to metal is throughout the range (inclusive) of about 80% to about 90%. In some situations, the ratio of carbon to metal (inclusive) is greater than 90%. The carbon to metal ratio can be affected (or further affected) by parameters or specifications (such as temperatures, thicknesses, homogeneity, etc.) that define the coating process.

FIG. 7 is a diagram 700 depicting a coating process. The figure refers to a metallic substrate, which substrate is subjected to plasma torch spraying of covetic materials, which in turn results in synthesized complex carbon coatings. The metallic substrate might comprise any one or more of copper, aluminum, or other bulk metallic materials. The covetic materials might comprise one or more of carbons, graphene, Nano-onions, carbon nanotubes (CNTs), carbide implanted materials, etc.

The plasma torch spraying serves to coat the input materials with deposited materials, and can be operated using pulsed energy. As shown, the deposited (such as by layer-on-layer sputtering) materials may be any one or more of carbon, metals (such as Al, Cu, Ti, Ta, etc.), and/or oxides or nitrides.

Several advantages emerge from use of the foregoing torches. Chiefly among them are the advantages of scalability and versatility of processes to formulate unique stable metal-carbon composites in a variety of configurations/architectures. These configurations/architectures range from fully dense thin film coatings to thick strips or particles for subsequent re-melting and casting/forming into engineered

metal alloy components. Each of these species throughout the aforementioned range exhibit unexpectedly favorable (and desirable) enhanced mechanical, thermal and electrical properties when compared to existing parent metal alloy formulations. Additionally, the tunability of the concentration and distribution of covalently-bound 2D graphene in a metal alloy matrix above the thermodynamic solubility threshold, and the layer-by layer formation in a non-equilibrium plasma environment, enables a new class of composite materials that can be engineered to correspond to a specific application and/or to correspond to specific property requirements. Moreover, this can be done at a significantly reduced cost as compared with other techniques.

The enhanced mechanical, thermal and electrical properties can apply to a large number of applications that use copper and aluminum alloys. As examples, such applications include (but are not limited to): wire conductors and high voltage power transmission cables, microelectronic thermal management and heat exchangers, and numerous applications that use thin film electrical conductors such as batteries, fuel cells, and photovoltaics. In particular, the combination of the microwave plasma torch process and enabling carbon-metal alloy production provides significant energy savings in manufacturing as well as increased thermal efficiency and reduced electrical losses in end-application performance.

The foregoing plasma spray techniques depict merely one genre of methods for making covetic materials. Another genre involves spraying carbon particles onto small molten metal particles. Such a genre and various species of that genre are shown and discussed as pertains to FIGS. 8A-B, FIG. 9, FIG. 10, FIG. 11, FIG. 12, FIG. 13, and FIG. 14, as well as in the discussions of the figures herein.

FIGS. 8A-B are schematics depicting a plasma spray process **800** that is used for spraying carbon particles onto small molten particles. As an option, one or more variations of the plasma spray process **800** (or any aspect thereof) may be implemented in the context of the architecture and functionality of the implementations described herein. The plasma spray process **800** or any aspect thereof may be implemented in any environment.

The shown plasma spraying techniques are used in various coating processes wherein heated materials are sprayed onto a surface. The feedstock (such as the coating precursor) is heated by electrical means (such as plasma or arc) and/or chemical means (such as via a combustion flame). Use of such plasma spraying techniques can provide coatings having a thickness in the range of about 20  $\mu\text{m}$  to about 3 mm, depending on the process and feedstock. The coating can be applied over a large area and at a high deposition rate. Using the foregoing techniques, the deposition rate is much higher than can be achieved by conventional coating processes such as electroplating or physical and chemical vapor deposition.

In addition (or in alternative) to the example materials above, the types of coating materials available for plasma spraying include metals, alloys, ceramics, plastics and composites. They are fed into the spray torch in powder form or in wire form, then heated to a molten or semi-molten state and accelerated towards substrates in the form of micrometer-size particles. Combustion or electrical arc discharge can be used as the source of energy for plasma spraying. Resultant coatings are made by the accumulation of numerous layers of sprayed particles. In many applications, the surface of the substrate does not heat up significantly, thus facilitating coating of many substances, including most flammable substances.

FIG. 9 is a scanning electron microscope image **900** showing the effect of spraying carbon particles (such as with particles sizes from 20 nm to 40 microns) onto small molten metal particles. The carbon particles sprayed onto small molten metal particles can be used in various specialized applications. For example, a plasma aluminum-graphite composite can be specially designed to provide coatings for turbine engines. Alternatives include use of aluminum and titanium alloys. The rate of growth of this plasma spray coating material is parabolic. The plasma spray coating material precipitates over short periods of time, which precipitation is largely independent of temperature. For preparation of the material surface, certain processes include preheating of the materials. In some implementations, blasting by grit is performed as well for preparation of the material surface. In some implementations, some portion of the particles that are sprayed onto the surface are still hot enough to form covetic bonds at the surface of the substrate. In other cases, small molten particles are at a temperature to form metal-to-metal bonds.

Use of the herein-disclosed microwave plasma torch techniques enables the creation of improved materials as compared to use of conventional torches. Specifically, power control limitations and other configuration constraints inherent to conventional plasma torches limit the ability of a conventional plasma torch to independently control input materials and other conditions needed to produce carbons that are effective in the creation of covetic materials that exhibit sufficiently high quality and homogeneity.

FIG. 10 shows a chart depicting a graphene growth temperature profile **1000** and a binary phase diagram. As an option, one or more variations of graphene growth temperature profile **1000** or any aspect thereof may be implemented in the context of the architecture and functionality of the implementations described herein. The graphene growth temperature profile **1000** or any aspect thereof may be implemented in any environment. The figure also shows a binary phase diagram, where the x-axis is the carbon concentration in a selected metal (such as copper, as shown) as expressed in atomic percent. The temperatures in the temperature profile in the figure as also shown in the phase diagram. Various metals can be used (such as silver, tin, etc.). In some cases, alloys are formed.

A general idea behind the growth of single layer graphene (SLG) or few layer graphene (FLG) on molten metal is to dissolve carbon atoms inside a transition metal melt at a certain temperature, and then allow the dissolved carbon to precipitate (referring to the creation of a solid from a solution) out at lower temperatures.

The schematic depicts graphene growth from molten nickel by (for example): (1) melting nickel while in contact with graphite (as carbon source), (2) dissolving the carbon inside the melt at high temperatures, and (3) reducing the temperature for growth of graphene.

As depicted, keeping the melt in contact with a carbon source at a given temperature will give rise to dissolution and saturation of carbon atoms in the melt based on the binary phase transition of metal-carbon. Upon lowering the temperature, solubility of the carbon in the molten metal will decrease and the excess amount of carbon will precipitate on top of the melt.

FIG. 11 is a cross-section view of a (conventional) plasma flame apparatus **1100**. The figure is being presented to distinguish uses of a legacy plasma flame apparatus as compared to uses of the herein-disclosed microwave plasma torch. Specifically, although use of a legacy plasma flame apparatus can produce diamond, or diamond-like materials

on the surface of metals, the process requires significant time for material dissolution of carbon and diffusion so that the final materials precipitate out onto the surface of the metal. During the creation of metal-carbon composite materials as disclosed herein with the presently disclosed implementations, graphene is desired to be interstitially grown and locked between layers (or within lattice or matrix sites) of metals or metal-containing composite materials. However, to do so, the temperatures must be modulated at a high rate. Unfortunately, legacy plasma torches do not offer sufficient control over the temperature and other conditions that are needed to reduce the size of interstitial carbon structures to the nanometer scale (as may be desirable in connection to achieving the covetous materials as desired herein).

In contrast, a pulsed microwave reactor (as relevant to the presently disclosed implementations as introduced earlier) and corresponding processes are shown and described in FIG. 12 to offer sufficient detailed control over the temperature and other conditions that are needed to reduce the size of interstitial carbon structures to the nanometer scale.

FIG. 12 depicts a pulsed microwave process flow 1200 that is used when “growing” graphene, referring to the layer-by-layer systematic deposition or application of graphene on substantially flat exposed surfaces of molten metal particles. As an option, one or more variations of pulsed microwave process flow 1200 or any aspect thereof may be implemented in the context of the architecture and functionality of the implementations described herein. The pulsed microwave process flow 1200 or any aspect thereof may be implemented in any environment.

When using the shown pulsed microwave process flow 1200, graphene is grown onto small molten particles. This is accomplished by interactions within the pulsed microwave reactor that occur around inlet 1204 (such as where the metal powder and carrier gas are inlet into the reactor chamber). In addition to inlet 1204, a process gas port 1202 and additional ports (such as additional port 12031 and additional port 12032) are provided at different heights on the side of the reactor apparatus. A waveguide traverses at least the distance from the position of the process gas port 1202 on the side of the reactor to the position of the inlet 1204 on the side of the reactor. Details of how to make and use ports for introduction and continued supply of material into such a reactor for growing graphene onto small molten particles are further disclosed below. More specifically, certain components of the reactor of FIG. 12 are shown and described as pertains to FIG. 13.

FIG. 13 is a perspective view of a conventional pulsed microwave plasma spray waveguide apparatus 1300 that is used for growing graphene onto small molten particles. As an option, one or more variations of pulsed microwave plasma spray waveguide apparatus 1300 or any aspect thereof may be implemented in the context of the architecture and functionality of the implementations described herein. The pulsed microwave plasma spray waveguide apparatus 1300 or any aspect thereof may be implemented in any environment.

In this implementation, microwave delivery components and a pulsing power supply are integrated to form a “surface-guide” (or the like) gas reactor. As shown, a combination of these components is configured to facilitate growing graphene onto small molten particles using a microwave plasma torch.

An alternative approach is to perform micro-welding using a tungsten inert gas (TIG) plasma source to partially or entirely melt the metal. Such a micro-welding technique is shown and described as pertains to FIG. 14.

FIG. 14 is a schematic depiction of a micro-welding technique 1400 that is used for growing graphene onto small molten particles. As an option, one or more variations of micro-welding technique 1400 or any aspect thereof may be implemented in the context of the architecture and functionality of the implementations described herein. The micro-welding technique 1400 or any aspect thereof may be implemented in any environment.

10 A low power, low flow TIG welder power supply and control unit with a custom plasma containment section can be effectively used to heat metal particles of all types. As shown, the exhaust plume, when inserted into the surface wave plasma gas dissociation tube, allows temperatures to remain high enough for the growth of graphene. This mode of growth involving control of plasma radicals composed of hydrocarbons and other added gases formed under non-equilibrium conditions provides many tuning opportunities that can be exploited by many different configurations of a 15 microwave plasma spray apparatus. FIG. 15, FIG. 18A1, FIG. 18A2, FIG. 18B, FIG. 18C, and FIG. 18D, as well as other figures and corresponding written description disclose example configurations of plasma spray apparatus.

FIG. 15 is a schematic depiction of a plasma spray 20 apparatus in a coaxial configuration 1500. As an option, one or more variations of coaxial configuration 1500 or any aspect thereof may be implemented in the context of the architecture and functionality of the implementations described herein. The coaxial configuration 1500 or any 25 aspect thereof may be implemented in any environment.

In a coaxial style implementation, microwave energy 30 delivery is achieved via TEM waves fed into an antenna with the outer portion of the coaxial member being a quartz tube outside of which are flowed powdered metallic particles. The gas that is fed into the center region in this example is a hydrocarbon gas such as methane, where it absorbs the 35 microwave radiation. The powder is heated by microwave energy that escapes the central region and by external inductive heating, which causes metal powder (in particulate form) to melt near the inclined portion, or tip, of the 40 displayed reaction chamber. As the CH<sub>4</sub> decomposes (into its constituent species, carbon, hydrogen, and/or derivatives thereof), carbon radicals nucleate on the surface of the melted metal droplets via the energy of the plasma radicals. Tuning of the microwave duty cycle, as well as tuning of the 45 inductive heating, as well as tuning of the plasma characteristics, facilitates maintenance of different temperatures between the melt and the plasma decomposition/ionization region. Moreover, the non-equilibrium temperature allows for (facilitates) internal lattice placement of the graphene/carbon, and quick quenching creates conditions conducive to further covetous materials growth.

FIG. 16 is a schematic depiction of a plasma spray 50 apparatus 1600 showing the evolution of materials by processing through a series of non-equilibrium energy conditions. As an option, one or more variations of the plasma spray apparatus 1600 (or any aspect thereof) may be implemented in the context of the architecture and functionality of the implementations described herein. The plasma spray apparatus 1600 or any aspect thereof may be implemented in any environment.

The figure depicts evolution of materials as they pass 55 through the apparatus. Specifically, the figure depicts the regions where different evolutionary changes occur such that in the region near the tip, graphene is grown onto the small metal melt particles. This material is deposited onto a substrate.

FIG. 17 depicts a surface wave plasma system 1700 for growing graphene onto molten particles. As an option, one or more variations of the surface wave plasma system 1700 or any aspect thereof may be implemented in the context of the architecture and functionality of the implementations described herein. The surface wave plasma system 1700 or any aspect thereof may be implemented in any environment.

In the shown configuration, the supply gas is fed into the center region of the apparatus. In this example a hydrocarbon gas such as methane is used. The hydrocarbon gas absorbs the microwave radiation, which provides a heat source to heat metal powder. Thus, the metal powder is heated from both: (1) the microwave energy that escapes the central region; and, (2) the external inductive heating, to melt and become molten near the tip. As the hydrocarbon gas decomposes, carbon radicals nucleate on the surface of the melted metal droplets via the energy of the plasma radicals.

FIG. 18A1 depicts an axial field configuration 1810 of a plasma spray torch. The formation of covetic materials has been discussed using several different apparatuses and corresponding processes. Any of the foregoing apparatuses and corresponding processes can be tuned to achieve particular conditions for formation of covetic materials. In the specific axial field configuration shown, the processes include generating an electric field 1804 between the electrodes to create current flow through a melt of metallic and carbon materials. Specifically, and as shown, a specially configured plasma torch has an externally controlled field where the melted particles form a plasma, which in turn becomes a meta electrode. The electrode on the other side of the field is formed by the shown growth plate 1803. The covetic materials are accelerated through an acceleration zone 1821 and then deposited onto a surface. The created alloy and covetic materials continue to be deposited onto the growth plate and/or onto previously deposited materials in the impaction zone 1823. This technique for deposition results in a material where the carbon loading is homogeneous and in high concentration.

Input materials can be selected and varied so as to achieve particular properties exhibited materials. For example, and as shown, inputs to the plasma spray torch may include various input gasses 1812 as well as input metallics and/or carbon particles 1818. The foregoing inputs can be introduced into one or more input ports 1862. In some cases, the input metallics and/or carbon particles are entrained within a flow of input gasses 1812. Furthermore, the growth plate can change its dimension and composition during ongoing deposition. For example, and as shown, the growth plate 1803 can initially be a substrate 1816, on top of which is deposited hot covetic materials in a torch stream that at least partially melts the substrate as the covetic materials are deposited. The deposited hot covetic materials cool from a molten or partially molten state to form quenched layers.

In this manner, any number of layers can be formed. The temperatures at the substrate and/or at or near the topmost layer can be controlled such that when a next layer of materials lands on the molten metal of the just formerly-deposited layer, the newly-deposited layer grows in a lateral way to produce single-layer graphene on the surface of this molten metal. This mechanism is distinguished from other techniques at least in that, in contrast to conventional metal melt methods 103, where carbon precipitates out of a molten metal slurry, application of the herein-disclosed plasma spray torch methods 104 results in quenching in a short time period such that there is insufficient time for the carbon to precipitate out of the matrix. Thus, covetic bonds remain

intact throughout the layer. A few moments later, after the quenching has formed a solid of metal and well dispersed carbon, another layer is sprayed on top of that, and so on, thereby forming layers of single-layer graphene that was grown, captivated and quick-quenched to produce a true covetic material with extremely high carbon loading within the matrix. As one example, when using conventional metal melt methods 103 (see FIG. 1A), carbon loading might achieve 6% carbon metal. In contrast, when using plasma spray torch methods 104 (see FIG. 1A), 60% carbon loading is readily achieved. In some cases, tight control of inputs and process parameters of the plasma spray torch and its environment allow carbon loading to approach as much as 90% carbon in the resulting material.

15 Experimental results using plasma spray torches have shown that highly loaded, highly uniform covetic layers can be formed by at least two quick-quench (such as 'splat') methods. A first method brings in carbon particles to cover metal particles (such as in the plasma) and the resulting hot mixture is sprayed onto a much cooler substrate. A second method creates graphene in the plasma and then brings in molten metal that covers the graphene. In both cases, true covetic (referring to a combination of covalent and metallic chemical) bonding occurs while in the plasma plume, and 20 the quick quenching of the spray serves to captivate the mixture into an organo-metallic lattice.

25 As shown in FIG. 18A2, the depth or thickness of the quenched layers 1824 can be caused to be thicker or thinner by controlling distances between the plasma flame 1814 and the substrate and/or by controlling the temperatures at the substrate 1816 (such as either higher or lower than ambient) and/or by controlling the pressures in and around the reactor.

30 FIG. 18B depicts a radial field configuration 1820 of a plasma spray torch. In this configuration, the melted particles form a plasma within the torch, which plasma becomes a meta electrode. The other electrode is formed by the side of the internal wall.

35 The foregoing configurations of FIG. 18A1, FIG. 18A2, and FIG. 18B are merely examples. Other configurations involving different input materials and different input port configurations are possible without departing from the generality of the plasma spray torch disclosed herein. Moreover, different configurations involving different input materials and different input port configurations can achieve the same 40 intended results. For example, two different configurations that are tuned to achieve the same resultant material are shown and described as pertains to FIG. 18C and FIG. 18D. Specifically, the example configurations of FIG. 18C and FIG. 18D can be used for plasma spray torch deposition of 45 ceramic film materials onto carbon-containing particles (such as graphene-containing particles).

50 Indeed, thin film deposition of carbon-containing materials (such as via atmospheric pressure chemical vapor deposition (APECVD) and/or other variations of chemical vapor deposition (CVD)) have made their way into many 55 areas of materials processing. Various composites and coatings involving such carbon-containing materials may exhibit improved physical properties (such as strength, imperviousness to corrosion, etc.). The morphological characteristics of various 2D and 3D carbons inure these improved physical 60 properties to the composites and coatings by virtue of molecular-level configurations within the carbon-containing materials. In some cases, use of 2D and 3D carbons in composites and coatings greatly increases the resultant carbon-containing material's imperviousness to high temperatures; however, in some cases, these high temperatures rise 65 above ~2100° C., which is high enough to burn the 2D and

3D carbons themselves. Unfortunately, destroying the 2D carbons and 3D carbons in turn destroys the benefit originally garnered by the carbons in the composite or coating. Therefore, deposition techniques (such as plasma spray torch configurations) are needed to create composites or coatings that are impervious to temperatures even higher than the combustion temperature of carbon.

FIG. 18C depicts such a configuration, strictly as a non-limiting example. By tuning the inputs and various in-reactor conditions, graphene-containing materials can be coated with a heat-absorbing layer of organically modified silicon (ORMOSIL). The deposition of ORMOSIL ceramic materials onto graphene-containing materials can be achieved via several methods including through the process of atmospheric, reactive plasma-enhanced chemical vapor deposition using a silicon-containing precursor 1841 (such as hexamethyl di-siloxane) and a reactive gas such as oxygen. This particular mixture of the silicon-containing precursor and oxygen is made reactive within the plasma. The molecular dissociation that occurs within the plasma flame leads to deposition of silicon oxide onto surfaces such as the foregoing growth plate 1803. To accomplish this, in-reactor conditions are controlled such that an organically modified silicon ceramic is deposited onto surfaces of carbon-containing particles as they form in the reactor. Control of in-reactor growth and in-reactor deposition (such as by controlling APECVD processes) leads to a thin quartz coating around the carbon-containing particles, which are in turn deposited onto a substrate. The thin quartz coating acts as a flame-retardant layer to protect the carbon-containing particles from burning at elevated temperatures.

FIG. 18D depicts an alternative configuration, strictly as a non-limiting example. As shown, metallic and/or carbon-containing materials are input into the reactor. Microwave energy 1822 is controlled to achieve at least the temperature to dissociate the carbon-containing materials (such as T(c-dis) of FIG. 10). A silicon-containing precursor 1841 (such as HMDSO, HMDSN, etc.) is introduced into the plasma flame and the temperature is lowered in the plasma afterglow. As the temperature is lowered, carbon particles begin to form, becoming coated with the silicon oxide. The carbon particles coated with the silicon oxide are then deposited onto a substrate.

In one implementation, a thin layer of perhaps 10 nm thick of these 3D materials can be deposited onto a substrate, which won't burn or catch fire even at 1200° C. This is because pristine carbon (such as graphene) is crystallized, such as it's not an amorphous material. Rather, it has been reduced to a state where it simply won't burn anymore.

On one use case, the foregoing plasma spray torch techniques can be used to produce new types of solder that is non-eutectic. Or, as another use case, the plasma spray torch can spray a coating of material directly onto a substrate to prevent the underlying material from oxidizing.

In addition to forming materials that do not combust even at 1200° C. in atmospheric pressures, putting quartz around materials often yields huge advantages in applications.

Besides organically modified silicon, other organic substances can be used to coat the carbon particles or the carbon layers. Characteristics of the coating can be controlled. As one example, the pores of the surface of the sprayed-on materials can be tuned to be hydraulically smooth.

A plasma spray torch can be used to form a heat-absorbing, glass-coated, non-flammable graphene composed of graphene and silicon, where the silicon coats the graphene such that the graphene is able to withstand temperatures

higher than 1600° C. Such a heat-absorbing, glass-coated, non-flammable graphene absorbs infrared energy.

One specific method for producing organically-modified silicon coatings comprises steps of (for example): (1) introducing a silicon-containing precursor into a plasma spray torch apparatus, (2) combining the silicon-containing precursor with a carrier gas having carbon particles that are entrained in the precursor gas, and (3) coating the carbon particles with silicon.

The characteristics of the flame-retardant and infrared obscurant materials that result from the plasma spray torch configuration of FIG. 18C and/or FIG. 18D can be tuned, at least in part, by controlling the time-temperature paths though the reactor. More generally, the characteristics of materials that result from the plasma spray torch configuration of FIG. 18A1, FIG. 18A2, FIG. 18B, FIG. 18C or FIG. 18D can be tuned, at least in part, by controlling (such as pulsing) the microwave energy within the reactor.

FIG. 19 is a chart 1900 that depicts energy versus time during pulse on and pulse off. More specifically, the chart shows one complete time cycle, from time T=0 through 50 microseconds with the microwave being continuously turned on, and then the remaining portion of the shown cycle depicts a time with the microwave being turned off. The plotted curves depict (1) changing density, and (2) changing temperature over the cycle. At time T=0, the temperature is at a minimum point (such as depicted at the origin of the chart). The temperature rises rapidly, then decreases, during which time the plasma density reaches a relatively stable value. When the microwave is turned off at time T=50 microseconds, both the plasma density and the temporal electron temperature decrease rapidly. The pulse time and duty cycle can be controlled so as to achieve a particular density and temperature at any point in time.

FIG. 20A1 depicts images that show organo-metallic bonding that occurs when combining carbon and copper using a plasma spray torch. As shown, carbon 2052 is deeply embedded within copper 2054. As commonly understood and as referred to herein, organometallic chemistry implies the study of organometallic compounds, chemical compounds containing at least one chemical bond between a carbon atom of an organic molecule and a metal, including alkaline, alkaline earth, and transition metals, and sometimes broadened to include metalloids like boron, silicon, and tin, as well. Aside from bonds to organyl fragments or molecules, bonds to 'inorganic' carbon, like carbon monoxide (metal carbonyls), cyanide, or carbide, are generally considered to be organometallic as well. Related compounds such as transition metal hydrides and metal phosphine complexes may be included in discussions of organometallic compounds, though strictly speaking, they are not necessarily organometallic.

Within organometallic chemistry, organocopper compounds contain carbon to copper chemical bonds, and may possess unique physical properties, synthesis, and reactions. Organocopper compounds may be diverse in structure and reactivity but remain somewhat limited in oxidation states to copper(I), such as denoted Cu<sup>+</sup>. As a d<sup>10</sup> metal center, it is related to Ni(0), but owing to its higher oxidation state, it engages in less pi-backbonding. Organic derivatives of Cu(II) and Cu(III) may be invoked as intermediates but are rarely isolated or even observed. In terms of geometry, copper(I) adopts symmetrical structures, in keeping with its spherical electronic shell. Typically, one of three coordination geometries may be adopted: linear 2-coordinate, trigonal 3-coordinate, and tetrahedral 4-coordinate. Organocop-

per compounds form complexes with a variety of soft ligands such as alkyl phosphines ( $R_3P$ ), thioethers ( $R_2S$ ), and cyanide ( $CN^-$ ).

By any one or more of the aforementioned techniques, the carbon depicted in FIG. 20A1 and FIG. 20A2 is chemically bonded to copper—as opposed to merely being juxtaposed to copper to adhere thereto via van der Waals forces (such as referring to a distance-dependent interaction between atoms or molecules). Unlike ionic or covalent bonds, van der Waals attractions do not result from a chemical electronic bond; they are comparatively weak and therefore more susceptible to disturbance. Moreover, the van der Waals forces quickly vanish at longer distances between interacting molecules. Instead, what is desired is organo-metallic bonding between a metal and carbon.

FIG. 20A2 depicts images that are a graded composition of matter applied into a substrate material and showing three material property zones. The bulk metal zone 2066 is a first material property zone of these three material property zones. As shown, the first material property zone comprises a metal in a first crystallographic formation, the first crystallographic formation having substantially metallic bonds between metal atoms present in the first material property zone. This first material property zone is substantially adjacent to a second material property zone that at least partially overlaps the first material property zone. The covetic material zone 2064 comprises at least some carbon atoms in a second crystallographic formation, wherein the second crystallographic formation has at least some covalent bonds between some of the carbon atoms that are present in the second material property zone and the metal atoms that are present in the first material property zone. The top surface zone 2062 is a third material property zone that at least partially overlaps the second material property zone. This top surface zone comprises further carbon atoms that are oriented in a third crystallographic formation. The third crystallographic formation is characterized as having at least some covalent bonds between individual ones of the further carbon atoms that are present in the third material property zone. In various implementations, there may be some metal atoms in any of the zones, and there may be some carbon atoms in any of the zones however, this implementation is characterized by a higher metal content zone 2074 that is adjoining to the bulk metal zone 2066. In various implementations, here may be some carbon atoms in any of the zones, and there may be some metal atoms in any of the zones however, this implementation is characterized by a higher carbon content zone 2072 that is adjoining to the top surface zone 2062.

FIG. 20B is a materials evolution chart 20B00 depicting several layered configurations that occur when adding carbon to bulk aluminum. In these implementations, materials are sprayed onto an existing, carbon rich covetic substrate or carbide layer to create a carbon to carbon bond through carbon sintering and/or metal melt encapsulation, which in turn creates attachments to form a composite film. The materials evolution chart 20B00 is merely one example of a combinational material (silicon carbide) that is sprayed onto an aluminum bulk material. The process can be tuned to create a covetic or covetic-like film that is deposited onto bulk materials. The resulting materials then can be coated to create a functionalized top layer. One possible configuration of an apparatus for spraying combinational material onto substrate is given in FIG. 21A.

FIG. 21A depicts an apparatus for spraying a molten mixture of materials onto a substrate. The figure depicts a microwave reactor that comprises multiple regions inside a

containment vessel. Pulsed microwave energy from microwave energy source 2117 operatively coupled to the reactor is delivered into the containment vessel. A hydrocarbon process gas 605 is provided through an inlet port. The microwave energy heats the process gas to a high enough temperature to form plasma. The expansion of materials within the containment vessel creates a plasma plume. The continuous addition of materials into the containment vessel in combination with the aforementioned expansion results in a torch effect in and around the plume. Resulting from the high temperatures within and around the plasma plume, the carbon dissociates from the hydrogen, thus forming several different hydrocarbon species (such as  $CH_3$ ,  $CH_2$ ). As the temperature continues to increase (such as in the first region 2104, as shown), all or nearly all of the carbon atoms become dissociated from the hydrogen. Using any known technique (such as using a gas-solid separator), the hydrogen-only species are separated from the solid carbon species.

At the interface between the first region 2104 of the containment vessel and the second region 2106 of the containment vessel, molten metal or molten metal composite, or molten ceramic-metal, or metal matrix, or metal mixture of any sort is introduced through a second inlet into the containment vessel (as shown). The location of the second inlet is selected based on the dimensions of the plasma plume, and/or the temperature of the molten metal at the point of inlet into the containment vessel. More specifically, the metal melt 2108 is introduced into the reactor at a location where the molten metal mixes with the carbon species. As the mixture flows (such as at a high rate of velocity) through the containment vessel, the mixture cools to a lower temperature. The flowing mixture exits the containment at a high rate of velocity such that the mixture of carbon and molten metal is sprayed out of the exit port 2110. The mixture is deposited (such as via spraying sprayed material 2112) onto a target substrate 2116. Various mechanisms for controlling the uniformity of the sprayed material 2112 and/or the resulting deposited material 2114 are shown and discussed as pertains to FIG. 23A through FIG. 23D.

The temperatures in the second region are low enough that at least some of the carbon precipitates out of the mixture. However, most of the dissociated carbon remains in mixture with the molten metal. When the molten metal mixed with the carbon reaches the target substrate 2116, it cools into a solid. During the transition from a molten mixture to a solid deposit, carbon is trapped between layers of metal and carbon. At certain temperatures the carbon forms covalent bonds with the metal, thus resulting in covetic material. This covetic material exhibits a range of mechanical, thermal, electrical and tribological properties due to increased cohesion forces (such as covalent bonds) between the metal matrix and carbon.

Such covetic materials are a result of use of the pulsed microwave energy to control the energy distribution of the constituents of the materials in the first region and second region of the reactor. More specifically, the energy distribution of the constituents of the materials in the first region and second region of the reactor can be controlled in part by pulsing the microwave and in part by pre-melting the metal particles in an environment external to the chamber of the reactor (such as so as to introduce fully-melted or partially melted metal into the reactor chamber). Any known techniques can be used, singly or in combination to melt the metal particles. As such the degree and/or mixture of fully melted or partially melted particles can be controlled.

FIG. 21B depicts a method for spraying covetic materials onto a substrate. The method can be used in conjunction with

the apparatus of FIG. 21A. As shown, the method is performed using a microwave reactor having an inlet for a process gas, an inlet for a metal melt, and an exit port. Prior to operation, the microwave reactors configured (operation 21B02). At operation 21B10, the inlet serves to introduce a hydrocarbon process gas into a first region of the reactor. Using the microwave energy, the temperature in the first region of the reactor is elevated such that the hydrocarbon process gas dissociates into carbon and hydrogen species before reaching the metal melt. A different inlet serves to introduce a metal melt into a second region of the reactor (operation 21B20). The elevated temperature in the second region is maintained until the dissociated carbon mixes with the metal melt (operation 21B30). The effect of the aforementioned plume operates to move the mixture into a third region of the reactor (operation 21B40). Movement away from the microwave energy source has the effect of reducing the temperature of the mixture until at least some of the carbon condenses out of the mixture (operation 21B50). However, even though the temperatures are reduced, the plasma torch effect serves to move the mixture through the exit port at a high rate of velocity (operation 21B60). As such, the molten mixture is sprayed onto a substrate (operation 21B70).

FIG. 21C is a schematic depicting a plasma spray process that is used for spraying a film. As shown, carbon radicals, polycyclic aromatics, graphene sheets, and metal particles are mixed at high temperatures in a plasma reactor (such as referring to the shown first region 2104). Nucleation occurs at these high temperatures, and as temperatures inside the reactor decrease (such as referring to the shown second region 2106), growth and assembly begins. One possible growth mechanism is depicted by the sub-micron sized aluminum particles being coated by few layer graphene. These sub-micron sized aluminum particles are held together with a combination of metallic bonds, covalent bonds and covetic bonds. More specifically, and as shown at the 2 nm scale, carbon atoms are bonded to aluminum atoms. The carbon atoms are organized into a coherent graphene plane that is situated in the aluminum matrix. The foregoing discussion involving aluminum is merely an example. Other metals can be used. In fact, a coherent graphene plane can be situated not only in a face-centered cubic (FCC) metal lattice, but also in a body-centered cubic (BCC) metal lattice, or in a hexagonal close packed (HCC) metal lattice.

The foregoing coated particles are then sintered to form particles that have diameters on the order of 100 microns. These semi-molten particles are then accelerated through the reactor and impacted onto a substrate (such as in a first pass), or onto a previously deposited layer of impacted particles (such as in a second or Nth pass).

FIG. 22A depicts an apparatus for wrapping carbon particles with a molten metal. The configuration of the apparatus of FIG. 22A differs from the configuration of the apparatus of FIG. 21A at least in that the introduction of the molten metal is controlled using the melting apparatus 2209. The metal melt is controlled so as produce molten metal that wraps around carbon particles when the molten metal is introduced into the reactor.

FIG. 22B depicts a method for wrapping carbon particles with a molten metal. The method differs from the method of FIG. 21B at least in that, in operation 22B30, the temperatures in the different regions of the reactors are maintained such that some carbon particle species form from the dissociated carbons. In operation 22B50, at least some of those carbon particles become wrapped by the molten metal. Some bonds are formed between constituent atoms of the

carbon particles and atoms of the metal melt. In operation 21B60, the metal-wrapped carbon particles moved through the exit port, further reducing the temperature. When the metal-wrapped particles are deposited onto the substrate (operation 21B70) further bonds are formed between the metal-wrapped carbon and the metal of the substrate.

FIG. 23A, FIG. 23B, FIG. 23C, and FIG. 23D depict example deposition techniques, according to some implementations.

As shown in FIG. 23A, the deposited material has a curved shape that is characterized by a middle region of a higher height and end regions of a lower height. In some cases, this is a desired shape for a spot of deposited material. In other cases, it is desirable to spray deposited materials over larger areas. This can be accomplished by moving the substrate with respect to the spray, or by moving the spray with respect to the substrate. FIG. 23B depicts a flexible substrate 2310 that is dispositioned onto a supply reel. The flexible substrate can be drawn onto and around a take-up reel. As such, and in the configuration of FIG. 23B, the spray deposits covetic materials uniformly onto the moving substrate. When the relative movement between the sprayed material 2112 and the substrate is controlled, the resulting deposited materials are of uniform thickness.

In some situations, it is desired to have a non-flat, but uniform patterning at the surface of the deposited materials. In such a situation, the movement of the substrate can be stepped through a series of discrete positions, thus resulting in the patterning of FIG. 23C. Additionally, or alternatively, a slotted antenna can be disposed between the sprayed material 2112 and the substrate. The slotted antenna functions by distributing the spray evenly across the lateral distance of the slotted antenna. Using such a slotted antenna, a single spot of sprayed material 2112 can have thickness and surface uniformity substantially as shown in FIG. 23D.

FIG. 24A and FIG. 24B depict conventional techniques for deposition of materials onto a substrate. As shown in FIG. 24A, a carbon agglomeration is held together through use of a binder (such as polymers). This results in weak binding at the interface between the carbon agglomeration and the substrate. FIG. 24B depicts a coating of carbon materials onto a substrate using a binder. Conventional deposition using binders suffers from peeling. Moreover, even when the surface of the substrate is mechanically pretreated and/or pretreated with deposition of binder material, the interactions between the substrate and the carbon agglomeration are weak.

As heretofore described, coatings based on deposition of materials onto a substrate using binders and/or using coating techniques (such as such as are shown and described as pertains to FIG. 24A and FIG. 24B) suffer from peeling, low strength properties and other undesirable mechanical properties. Improvements based on plasma spray techniques are shown and discussed in FIG. 25A and FIG. 25B.

FIG. 25A and FIG. 25B depict example deposition techniques that result in covalent bonding at the surface of a substrate, according to some implementations. Specifically, and as shown, when the herein-disclosed techniques are used, covetic materials are formed by covalent bonds between the carbon and the substrate. As such, no binder is needed or used. Furthermore, many of the bonds formed at the interface between the substrate and the covetic material are strong covalent bonds. In one specific case, where the substrate is aluminum, covalent bonds are formed between atoms that are in the face-centered cubic structure of alu-

minum and atoms of carbon that are in a hexagonal structure. A schematic of interfacial bonding is depicted in FIG. 25B.

FIG. 26A, FIG. 26B, FIG. 26C, and FIG. 26D present schematic diagrams that depict how covalent bonds are formed between sites in the square shapes of a face-centered cubic structure of aluminum and sites in the hexagonal shapes that occur in certain crystallographic structures of carbons.

FIG. 26A is an orthogonal view showing the square shapes of face-centered cubic structure of aluminum. FIG. 26B is an orthogonal view showing the hexagonal shapes that occur in certain crystallographic structures of aluminum.

FIG. 26C depicts one possible superposition of the hexagonal shapes that occur in certain crystallographic structures of carbons on top of the square shapes of face-centered cubic structure of aluminum. FIG. 26D depicts covalent bonds that are formed at certain sites. The example of the face-centered cubic structure of aluminum is merely one example. Other metals having other crystallographic structures are possible.

FIG. 26E is an example of a layered covetic material 26E00, where a graphene-like structure is sandwiched between layers of metal material. The lower layer of metal material is a layer of substrate. The top layer of metal material is formed of quenched material that was formerly molten while in the reactor. The graphene-like structure that is sandwiched between layers of metal material is captured between the two layers of metal due to the formation of metal-to-metal bonds between the two metal layers. In addition to the metal bonds, other bonds are formed that serve to encase the graphene-like material between the metal layers. In some locations, there are defects in the carbon lattice. Various types of bonds are formed between or near such defects.

Any or all of the foregoing techniques for forming covetic materials can be used in many applications involving many different types of substrates. Moreover, the relative movement between the spray and the substrate can be controlled so as to result in deposits of any thickness. Any known techniques can be used to control the relative movement. For example, the exit port can be moved over a stationary substrate. This can be accomplished using a hand-held device or a robotically controlled device that is moved relative to the stationary substrate. In some cases, the substrate can be subjected to a bias voltage such that at least some of the material that is sprayed out of the exit port is electrostatically attracted to the surface of the substrate. This has applicability in applications where the substrate is not uniformly flat. As examples, applications where the substrate is not uniformly flat may include: (1) shaped components that are used in machinery that is subjected to corrosively harsh conditions, (2) turbine blades, (3) heat exchanger components, etc., many of which applications are further discussed infra.

In other situations, characteristics (such as thickness, lateral uniformity, etc.) of the deposition can be enhanced through use of and/or combinations of various chemical vapor deposition techniques. Strictly as one example, aspects or parameters pertaining to known-in-the-art plasma enhanced chemical vapor deposition techniques can be controlled so as to optimize characteristics of the deposited layers of covetic materials. As another example, rather than depositing covetic materials onto a surface to form a film or coating, covetic materials can be formed into particles (such as by spraying into a lower temperature environment) and

collecting the particles as a powder. Various techniques involving production and use of powdered covetic materials are briefly discussed hereunder.

#### Powdered Covetic Materials

In some situations, rather than forming covetic materials as a film or coating on or in a substrate, covetic materials can be delivered as a covetic material powder. Such a powdered covetic material can be collected as it exits the reactor, cooled to a temperature below the melting point of the covetic material and collected as a powder. The powder in turn can be handled (such as stored and shipped, poured, mixed, etc.) at room temperatures. The powder can then be remelted and pressed into a form or remelted and re-sprayed. As examples, components for use in highly corrosive environments can be formed from such powdered covetic materials using injection molding or extrusion. Many apparatuses can be used, singly or in combination to form and transport covetic material powders. Example apparatus are shown and described as pertains to FIG. 27A, FIGS. 27B1 and 27B2.

FIG. 27A depicts an example apparatus 27A00 for producing powdered covetic material 2710 using a cooling region 2702 to cool the sprayed material 2112 when the spray is forced through an exit port 2110 of a microwave reactor. Any one or more cooling techniques in any combination can be used to lower the temperature of the covetic material in cooling region 2702 to a temperature that is lower than the melting point of the covetic material. The cooling region 2702 might host one or more apparatuses to cause the cooling. For example, and as shown, a collection vessel 2704 might be fitted with one or more apparatuses to cause a cyclone effect in the collection vessel, thereby increasing the time for lowering the temperature of the covetic material. In some cases, the time for cooling the covetic material is controlled (such as by increasing or decreasing the time) so as to allow the covetic material to anneal with highly regular bonding. In some cases, controlling the time during which the covetic material is cooled allows for the covetic material to crystallize into highly regular crystalline structures, while still remaining in powdered form. In some implementations, a mechanical tumbler-agitator can be fitted between the exit port 2110 of the microwave reactor and collection vessel 2704. The tumbler-agitator can be cleaned or replaced periodically.

Alternatively, or additionally, and in situations where it is convenient and/or necessary to contain and/or transport powdered covetic material in a fluid, a fluidized bed apparatus can be used. For example, to avoid agglomeration of particles of the powder, the powdered covetic material can be held in a liquid. In some implementations, a fluidized bed apparatus can be fitted between the exit port 2110 of the microwave reactor and collection vessel 2704. One implementation of such a fluidized bed apparatus is shown and described as pertains to FIG. 27B1 and FIG. 27B2.

FIG. 27B1 and FIG. 27B2 depict an example fluidized bed apparatus 27B00 for cooling and handling powdered covetic materials in a fluid.

As shown, the molten metal and carbon mixture is forced through the exit port of the reactor and into the top of a fluidized bed 2750. As the molten metal and carbon mixture is forced out of the exit port, it is cooled in a manner that form particles. The particles are acted on by a downward force of gravity (such as in a downward direction, as shown) while at the same time a process fluid 2754 is forced from the bottom of the fluidized bed to create an upward force. As such, the particles accelerate toward the bottom of the fluidized bed at an acceleration rate slower than that of the local gravity. The flow dynamics can be partially modulated

by the geometry of the fluidized bed. For example, and as shown, a length of the fluidized bed can form a tapered body **2762** where a first end of the tapered body has a first dimension D1 and where a second end of the tapered body has a second dimension D2, and wherein D1>D2. The temperature within various portions of the fluidized bed can be controlled in part by power source **2752** that powers a coil (as shown) and/or by a heat source **2760** that heats process fluid **2754** before the process fluid enters the bottom of the fluidized bed.

The pressures and flow rates and other conditions in the fluidized bed and at the environmental interfaces of the fluidized bed serve to cause the powder and fluid mixture to behave together as a fluid. The mixture exhibits many properties and characteristics of fluids, such as the ability to free flow under gravity, and/or to be pumped using fluid handling technologies.

In the implementation of FIG. 27B1 and FIG. 27B2, the fluidized bed has multiple ports that are positioned at different heights of the tapered body. This is so that a first powder in fluid **27561** flows out at a particular temperature/pressure, whereas a second powder in fluid **27562** flows out at a second, different particular temperature/pressure. The flows through the multiple ports can be controlled such that the collection vessel can receive any ratio or amounts of first powder in fluid **27561** and second powder in fluid **27562**.  
Method of Forming Covetous Materials

Table 3 shows some non-limiting examples of methods for forming powdered covetous materials.

TABLE 3

| Example Methods  | Designation                                                                                                                         |
|------------------|-------------------------------------------------------------------------------------------------------------------------------------|
| Example Method 1 | Producing organo-metallic materials after dissociation of a hydrocarbon process gas in a microwave reactor-based plasma spray torch |
| Example Method 2 | Growing carbon allotropes on input particles within a microwave reactor                                                             |
| Example Method 3 | Coating input materials after dissociation of alternative process gases in a microwave reactor-based plasma spray torch             |

#### Example Method 1

In some implementations of method 1, structured carbons (such as carbon allotropes) are formed in a first region of a microwave reactor (such as through the dissociation of a hydrocarbon process gas). In a second region that is at a lower temperature than the first region, the structured carbons are decorated with a metal so as to form a metalized carbon material (such as an organo-metallic material). The metalized carbon material is further cooled to a temperature below the melting point of the metal. In some implementations, the metalized carbon material is initially in the form of carbon particles that are decorated with a metal. The particles are further cooled so as to form a powder. The powder can be collected and transported to an application facility. The powder comprising metalized carbon material having covetous bonds can be remelted and used in conjunction with any known techniques for forming a component from a powder. Strictly as examples, components can be formed from a powder by using die pressing followed by re-melting, isostatic pressing followed by re-melting, hot forging, metal injection molding, laser sintering, etc.

#### Example Method 2

In this method 2, one or more hydrocarbon gases (or in some cases gases and liquids) are input into the system.

Strictly as examples, the gases and/or liquids that can be input into the system include methane, ethane, methylacetylene-propadiene propane (MAPP), and hexane. In a first region **2104** at a first temperature, the carbon atoms are dissociated from other atoms (such as dissociated from hydrogen). A molten metal **2108** is introduced into the reactor as metal particles. Then, in a second region **2106**, the carbons produced in the first region combine with the metal particles. The carbon can grow on the surface of the metal particles and/or grow within the interior of the metal particles. In some situations, and under some conditions, the carbon growth comprises growth of 2D carbons on or in the metal particles. In other situations, and/or under other conditions, the carbon growth comprises growth of 3D carbons on or in the metal particles. In any of the foregoing growth situations, the growth can take place to the maximum extent allowed by the lattice. For example, the molten metal can be aluminum with a face-centered cubic (FCC) crystal structure, and the carbon can form a solid solution with the aluminum up to a particular concentration. In some implementations, the carbon forms a solution with the metal up to a concentration determined by the metal properties (such as the crystal structure) and then precipitate out of the metal-carbon solution to form 2D or 3D carbon on and/or within the metal particles.

The growth in this method 2 is carried out under non-equilibrium thermal conditions. Specifically, various differing thermal conditions to control (for example): (1) first temperatures (such as higher temperatures) in the first region that are needed to control the foregoing dissociation, and (2) second temperatures (such as lower temperatures) in the second region to control insipient melting of metal powders and/or the formation and properties of the metal-carbon particles in the second region. Temperatures in these two zones can be independently controlled. Using this method, the sprayed materials are true covetous materials that exhibit true covetous behaviors.

#### Example Method 3

In still further non-limiting examples, materials and/or coatings on input particles can be created or deposited from mixed materials such as trimethylamine (TMA), trimethylglycine (TMG), and methylacetylene-propadiene propane. The particles can be cooled and collected as a powder. Some examples of particles that can be created from target materials in the first zone are phased carbons, silicon carbide, metal oxides, metal nitrides or metals. In some cases, the input particles are metals, and compound films (such as metal oxides or metal nitrides) are coated on the metallic input particles, while in other cases, the input particles contain compound materials and metallic coatings are deposited on the input particles. Some examples of particles that can be created from input gases in the first zone are carbon allotropes (such as innate carbons), silicones, ZnO, AlOx, and NiO.

In some implementations, gases, including various non-hydrocarbon gasses or alcohols are input into the first zone and the first zone comprises a sputtering apparatus and a power supply, wherein the sputtering apparatus is configured to generate a plurality of ionic species from a selected target material. The target material and the ionic species combine to form a plurality of particles. The power supply can be an AC, DC, RF, or high-power impulse magnetron sputtering (HIPIMS) power supply and can be configured to generate a plurality of ionic species from the target material by tuning

the power, voltage, frequency, repetition rate, and/or other characteristics of the power supply.

FIG. 27C is a schematic depicting a plasma spray process that is used for production of a powdered covetic material. Powdered Material Processing Sequence

A visual representation of an example powdered material processing sequence from hydrocarbon cracking and particle nucleation (such as the shown first region 2104), to graphene growth (such as the shown second region 2106), cooling of the semi-molten particles (such as in the shown cooling region) and collection of powdered covetic material (such as in the collection region, and into the collection vessel 2104) is shown in FIG. 27C. Mechanisms that underlie the efficacy of the example powdered material processing sequence are now briefly discussed.

In absence of a metal precursor (whether metalorganic or particle form), the microwave plasma dissociates methane to form carbon radicals (as well as polycyclic aromatics/ acetylene) that will then form few layer (FL) graphene (or stacked lamellae) structures respectively. However, in the presence of a metal precursor in the plasma zone (such as refer to the reactors of FIG. 21A and FIG. 22A), the metal (either from metalorganic nuclei or particle) can serve as a seed site for heterogeneous carbon growth (such as carbon in the form of ionized radical, graphene nuclei, or polycyclic aromatic (acetylene)).

When using metals with a low solubility, such as Al or Cu, graphene sheets can grow (such as either through adatom/ monomers or as a cluster) onto the surface of the metal. Characteristics of the growth depends at least in part on symmetry and minimization of interfacial free energy at the metal surface. As such, carbon growth occurs at the metal particle alongside metal atom re-sputtering events at the surface to create intermixed and/or layered metal/carbon structures. As is known in the art, the radius of the metal particle (such as surface curvature), can affect carbon solubility in the metal particle. As an example, a smaller radius (such as corresponding to higher curvature) increases the solubility over equilibrium (at a planar surface), which increase in the solubility can in turn impact the thickness of the graphene layers.

Once the powdered covetic materials 2710 have been collected in a collection vessel, the powdered covetic materials can be further processed using conventional techniques (such as injection molding techniques, other techniques using powdered metal).

#### Manufacturing Techniques Using Powdered Covetic Materials

FIG. 28 depicts method for making components from powdered covetic materials using injection molding techniques. As shown, the method is initiated upon gathering a set of properties for a component to be used in a particular application and/or environment (operation 2810), then selecting a particular powdered covetic material based on at least one of the properties for the application or environment (operation 2820). The selection may be based on desired mechanical properties for the component, and/or based on desired anti-corrosive properties of the component in the environments corresponding to its intended use, and/or other desired properties. The selection might be based on multiple desired properties, and in some cases a selection tool solved an optimization problem based on a set of properties and an objective function.

Once the covetic material has been selected (operation 2820), the selected powdered covetic material 2825 is melted (operation 2830) and introduced into a mold (operation 2840). A prescribed temperature and a prescribed pres-

sure are maintained inside the mold for a prescribed duration (operation 2850) after which duration the temperature and pressure inside the mold is brought to about 30° C. and about atmospheric pressure (operation 2860). The component is released from the mold (operation 2870) and deployed in the intended application (operation 2880).

As heretofore mentioned, the selection of a particular covetic material might be based on multiple desired properties, some of which properties might be used as a variable of an objective function. In some cases, the selection of a particular covetic material might be based on a particular dominant property (such as mechanical strength, weight, anti-corrosiveness, etc.). In some cases, the properties of interest are ratios of other properties, such as strength to weight, specific heat to weight, etc.) In some cases, the dominant property is to be maximized (or minimized) subject to one or more constraints on other properties.

As such, powdered covetic materials can be deployed in a wide range of applications. In many cases, the resulting components made from powdered covetic materials outperform components made from other materials. Some example applications that correlate to certain dominant properties are shown and discussed as pertains to the following FIG. 29.

FIG. 29 depicts various properties of covetic materials. The shown properties include mechanical attributes, thermal conductivity, resistance to oxidation, durability, resistance to softening at high temperatures, resistance to fatigue, and electrical conductivity. Individual ones and/or combinations of these parameters become dominant when selecting a particular covetic material for a particular application.

Strictly as an example, resistance to oxidation might be a dominant parameter when selecting a covetic material for use in making corrosion-resistant valves. As another example, when selecting particular covetic materials to be used in the manufacture of blades for aircraft engine turbines, mechanical attributes such as a strength-to-weight ratio, subject to a strength minimum constraint might be a dominating mechanical attribute. The blade might also need to exhibit a very high resistance fatigue.

Typically, covetic materials exhibit not only the aforementioned properties but also are less dense than the metal or alloy that is used in making the covetic powder. A lower density often corresponds to a lower weight for a formed component as compared with the same component made from the metal or alloy in absence of carbon loading. As such, truck parts (such as cab components, as shown), automobile parts (such as doors fenders, roof panels, etc.), motorcycle parts, bicycle parts as well as various components (such as structural members) of airborne vehicles, and/or watercraft, and/or space-based vehicles or platforms can avail of the lower weight-to-strength ratio of covetic materials as compared with the base metals or alloys that are used in making the covetic materials.

As another example, covetic materials often exhibit exceptional thermal conductivity such that structural members formed of covetic materials can be used in high-temperature applications (such as heat sinks for electronics, industrial heat exchangers, etc.).

As yet another example, covetic materials often exhibit exceptional resistance to corrosion. More specifically, covetic laminates made using the foregoing techniques exhibit extremely high corrosion resistance, even at the top layer (such as at the component-to-environment interface). This property is of particular interest when components made with covetic materials are subjected to harsh environments.

As a still further example, covetic materials can be tuned for surface smoothness. More specifically, covetic laminates

## 39

made using the foregoing techniques exhibit extremely high surface smoothness. This surface smoothness property is of particular interest when the covetic materials serve as a heat shield, such as may be demanded in applications where friction at the surface (such as friction generated as a fluid passes over the surface at high speed) generates unwanted heat at the surface. By using the herein-disclosed techniques, the specific composition of the covetic material and/or by using the herein-disclosed specific techniques for deposition of the covetic material can result in a hydraulically smooth surface, which can in turn be used in airborne and/or space-based vehicles.

In certain implementations, one set of properties may dominate other properties. For example, the surface of a space-based vehicle (such as a satellite) might be required to be substantially non-reflective to a range of electromagnetic radiation (such as substantially non-reflective to visible light), while at the same time, the surface of the space-based vehicle might be required to be thermally isolating (such as thermally non-conducting). The foregoing tuning techniques accommodate such situations where a particular desired property (such as non-reflectivity) dominates the tuning of the plasma spray torch so as to produce a substantially non-reflective surface, even at the expense of other properties.

The properties as shown and described as pertains to FIG. 29 are merely examples. Additional properties and/or combinations of properties might be demanded or desirable in various applications, and these additional properties are exhibited in resultant materials based on tuning of inputs and controls of the plasma spray torch. Strictly as examples of the foregoing additional properties, such properties and/or combinations of properties might include or be related to a strength-to-weight metric, and/or a specific density, and/or mechanical toughness, and/or sheer strength, and/or flex strength, etc.

In the foregoing specification, the disclosure has been described with reference to specific implementations thereof. It will however be evident that various modifications and changes may be made thereto without departing from the broader spirit and scope of the disclosure. For example, the above-described process flows are described with reference to a particular ordering of process actions. However, the ordering of many of the described process actions may be changed without affecting the scope or operation of the disclosure. The specification and drawings are to be regarded in an illustrative sense rather than in a restrictive sense.

What is claimed is:

1. An apparatus for producing covetic materials comprising:  
a microwave energy source configured to generate pulsed microwave energy;

## 40

a reactor disposed in communication with the microwave energy source, the reactor comprising:

a first region configured to receive a hydrocarbon gas fed through a first inlet port and the microwave energy to dissociate the hydrocarbon gas into carbon and hydrogen species;

a second inlet port disposed downstream of the first region and configured to feed a metal melt into the reactor; and

a second region disposed downstream of the first region and in fluid communication with the second inlet port, the second region configured to form carbon particles from the dissociated carbon species and to produce a mixture of molten metal and carbon particles; and

an exit port configured to output the mixture of molten metal and carbon particles and form covetic materials as the mixture cools leaving the exit port.

2. The apparatus of claim 1, wherein the metal melt comprises one or more of aluminum, copper, or silver.

3. The apparatus of claim 1, wherein a temperature of the first region is greater than a temperature of the second region.

4. The apparatus of claim 1, further comprising a melting apparatus to form the metal melt, wherein the melting apparatus comprises a tungsten inert gas (TIG) welder power supply and control unit configured to melt metal powder in a plasma of inert gas.

5. The apparatus of claim 1, further comprising one or more of a cyclone apparatus, a mechanical tumbler agitator, or a fluidized bed apparatus disposed downstream of the exit port.

6. The apparatus of claim 5, wherein the one or more of the cyclone apparatus, the mechanical tumbler agitator, or the fluidized bed apparatus is configured to cool the mixture of molten metal and carbon particles.

7. The apparatus of claim 1, wherein the metal melt comprises one or more of a molten metal, a molten metal composite, a molten ceramic-metal, or a metal matrix.

8. The apparatus of claim 1, wherein the metal melt comprises one or more of fully-melted metal or partially melted metal.

9. The apparatus of claim 1, wherein the metal melt comprises metal droplets.

10. The apparatus of claim 1, wherein the covetic materials comprise sub-micron size metal particles and few layer graphene (FLG).

11. The apparatus of claim 1, wherein the covetic materials comprise graphene planes disposed in the metal matrix.

12. The apparatus of claim 1, wherein a pressure inside the reactor is at least 20 Torr.

\* \* \* \* \*